# EUROPEAN PATENT SPECIFICATION

(11) **EP 0 682 145 B1**
(45) Date of publication and mention of the grant of the patent: **25.08.2004**
(21) Application number: 95810288.1
(22) Date of filing: 03.05.1995
(51) Int. Cl.: D06L 3/12, D06P 1/64, C11D 3/42, C11D 1/62

(54) **Textile treatment**
Textilbehandlungen
Traitement textile

(30) Priority: 12.05.1994 GB 9409465; 12.05.1994 GB 9409466; 01.07.1994 GB 9413270
(43) Date of publication of application: 15.11.1995
(73) Proprietor: Ciba Specialty Chemicals Holding Inc., 4057 Basel (CH)
(72) Inventor: Reinehr, Dieter, Dr., D-79400 Kamdern (DE); Eckhardt, Claude, Dr., F-68400 Riedisheim (FR); Kaufmann, Werner, Dr., CH-4310 Rheinfelden (CH); Fankhauser, Peter, Dr., CH-4107 Ettingen (CH); Hilfiker, Rolf, Dr., CH-4054 Basle (CH)

(56) References cited:
- EP-A- 0 074 590
- EP-A- 0 275 694
- EP-A- 0 359 039
- EP-A- 0 508 744
- EP-A- 0 583 888
- EP-B- 0 240 461
- WO-A-94/04515
- WO-A-94/11480
- US-A- 4 009 193
- US-A- 4 309 316
- US-A- 4 339 393
- US-A- 4 460 485
- US-A- 4 478 598
- US-A- 4 539 161
- US-A- 4 772 404
- DATABASE WPI Section Ch, Week 8447 Derwent Publications Ltd., London, GB; Class D22, AN 84-291651 XP002062576 & JP 59 179 878 A (HOGI SHOTEN KK)
- DATABASE WPI Section Ch, Week 9349 Derwent Publications Ltd., London, GB; Class E19, AN 93-393176 XP002062578 & JP 05 295 603 A (TOYOBO KK)
- DATABASE WPI Section Ch, Week 9133 Derwent Publications Ltd., London, GB; Class A23, AN 91-242625 XP002069893 & JP 03 158 103 A (ORIDO ENGI KK)

## Description

The present invention relates to a use of a fluorescent whitening agent in a composition for improving the sun protection factor (SPF) of textile fibre material, wherein said fluorescent whitening agent absorbs radiation in the wavelength range 280-400 nm.

US-A-4 460 485 discloses fluorescent whitening agents, which are applied to textile fiber material. US-A-4 339 393 discloses distyrylbiphenyls as fluorescent whitening agents for textiles.

It is known that light radiation of wavelengths 280-400 nm permits tanning of the epidermis. Also known is that rays of wavelengths 280-320 nm (termed UV-B radiation), cause erythemas and skin burning which can inhibit skin tanning.

Radiation of wavelengths 320-400 nm (termed UV-A radiation) is known to induce skin tanning but can also cause skin damage, especially to sensitive skin which is exposed to sunlight for long periods. Examples of such damage include loss of skin elasticity and the appearance of wrinkles, promotion of the onset of erythemal reaction and the inducement of phototoxic or photoallergic reactions.

Any effective protection of the skin from the damaging effects of undue exposure to sunlight clearly needs to include means for absorbing both UV-A and UV-B components of sunlight before they reach the skin surface.

Traditionally, protection of exposed human skin against potential damage by the UV components in sunlight has been effected by directly applying to the skin a preparation containing a UV absorber. In areas of the world, e.g. Australia and America, which enjoy especially sunny climates, there has been a great increase in the awareness of the potential hazards of undue exposure to sunlight, compounded by fears of the consequences of alleged damage to the ozone layer. Some of the more distressing embodiments of skin damage caused by excessive, unprotected exposure to sunlight are development of melanomas or carcinomas on the skin.

One aspect of the desire to increase the level of skin protection against sunlight has been the consideration of additional measures, over and above the direct protection of the skin. For example, consideration has been given to the provision of protection to skin covered by clothing and thus not directly exposed to sunlight.

One aspect of the desire to increase the level of skin protection against sunlight has been the consideration of additional measures, over and above the direct protection of the skin. For example, consideration has been given to the provision of protection to skin covered by clothing and thus not directly exposed to sunlight.

Most natural and synthetic textile materials are at least partially permeable to UV

Most natural and synthetic textile materials are at least partially permeable to UV components of sunlight. Accordingly, the mere wearing of clothing does not necessarily provide skin beneath the clothing with adequate protection against damage by UV radiation. Although clothing containing a deeply coloured dye and/or having a tight weave texture may provide a reasonable level of protection to skin beneath it, such clothing is not practical in hot sunny climates, from the standpoint of the personal comfort of the wearer.

There is a need, therefore, to provide protection against UV radiation for skin which lies underneath clothing, including lightweight summer clothing, which is undyed or dyed only in pale shades. Depending on the nature of the dyestuff, even skin beneath clothing dyed in some dark shades may also require protection from UV radiation.

Such lightweight summer clothing normally has a density of of less than 200 g/m and has a sun protection factor rating between 1.5 and 20, depending on the type of fibre from which the clothing is manufactured.

The SPF rating of a sun protectant (sun cream or clothing) may be defined as the multiple of the time taken for the average person wearing the sun protectant to suffer sun burning under average exposure to sun. For example, if an average person would normally suffer sun burn after 30 minutes under standard exposure conditions, a sun protectant having an SPF rating of 5 would extend the period of protection from 30 minutes to 2 hours and 30 minutes. For people living in especially sunny climates, where mean sun burn times are minimal, e.g. only 15 minutes for an average fair-skinned person at the hottest time of the day, SPF ratings of at least 20 are desired for lightweight clothing.

Surprisingly, it has now been found that treating a textile fibre material with a fluorescent whitening agent which can also serve as a UV (ultra-violet) radiation absorber, namely one which absorbs radiation in the wavelength range 280-400 nm, in a composition, imparts an excellent sun protection factor to the fibre material so treated.

Accordingly, the present invention provides a use of a fluorescent whitening agent for improving the sun protection factor (SPF) of textile fibre material, wherein said fluorescent whitening agent absorbs radiation in the wavelength range 280-400 nm, in a composition, which is
a) an aqueous textile finishing composition;
   comprising at least one fluorescent whitening agent which is selected from the group consisting of bis-(triazinylamino)-stilbene-2,2'-disulfonic acid, 4,4'-bis-(triazol-2-yl)stilbene-2,2'-disulfonic acid, 4,4'-(diphenyl)-stilbenes, 4,4'-distyryl-biphenyl, 4-phenyl-4'-benzoxazolyl-stilbene, stilbenyl-naphthotriazoles, 4-styryl-stilbene, bis-(benzoxazol-2-yl) derivatives, bis-(benzimidazol-2-yl) derivative, coumarine, pyrazoline, naphthalimide, triazinyl-pyrene, 2-styryl-benzoxazole- or -naphthoxazole derivative, benzimidazole-benzofuran or oxanilide derivative, or
b) a detergent composition
   comprising at least one fluorescent whitening agent, which is selected from the group consiting of: in which R₄₃ and R₄₄, independently, are OH, NH₂, O-C₁-C₄-alkyl, O-aryl, NH-C₁-C₄-alkyl, N(C₁-C₄-alkyl)₂, N(C₁-C₄-alkyl)(C₁-C₄hydroxyalkyl), N(C₁-C₄-hydroxyalkyl)₂, NH-aryl, morpholino, S-C₁-C₄-alkyl(aryl), Cl or OH; R₄₅ and R₄₆, independently, are H, C₁-C₄-alkyl. phenyl or a group of formula: R₄₇ is H, Cl or SO₃M; R₄₈ is CN, SO₃M, S(C₁-C₄-alkyl)₂ or S(aryl)₂; R₄₉ is H, SO₃M, O-C₁-C₄-alkyl, CN, Cl, COO-C₁-C₄-alkyl, or CON(C₁-C₄-alkyl)₂; R₅₀ is H, C₁-C₄-alkyl, Cl or SO₃M; R₅₁ and R₅₂, independently, are H, C₁-C₄-alkyl, SO₃M, Cl or O-C₁-C₄-alkyl; R₅₃ is H or C₁-C₄-alkyl; R₅₄ is H, C₁-C₄-alkyl, CN, Cl, COO-C₁-C₄-alkyl, CON(C₁-C₄-alkyl)₂, aryl or O-aryl;
   and
   M is H, Na, K, Ca, Mg, ammonium, mono-, di-, tri- or tetra- C₁-C₄-alkyl ammonium, mono-, di- or tri-C₁-C₄-hydroxyalkylammonium or ammonium that is di- or tri-substituted by a mixture of C₁-C₄-alkyl and C₁-C₄-hydroxyalkyl groups, and n is 0 or 1;
   or
c) a post-wash fabric care composition comprising at least a fluorescent whitening agent, wherein said fluorescent whitening agent is a cationic bistyrylphenyl fluorescent whitening agent of formula:
in which Y is arylene, optionally substituted by chloro, methyl or methoxy; q is 1 or 2; R₅₅ is hydrogen, chloro, C₁-C₄-alkyl, C₁-C₄-alkoxy, cyano or C₁-C₄-alkoxycarbonyl; R₅₆ and R₅₇ are C₁-C₄-alkyl, chloroethyl, methoxyethyl, beta -ethoxyethyl, beta -acetoxyethyl or beta -cyanoethyl, benzyl or phenylethyl; R₅₈ is C₁-C₄-alkyl, C₂-C₃-hydroxyalkyl, beta -hydroxy- gamma -chloropropyl, beta - cyanoethyl or C₁-C₄-alkoxy-carbonylethyl; and An(⁻) is an anion of an organic or inorganic acid; or, a cationic bistyrylphenyl fluorescent whitening agent of formula: in which R₅₅ and q have their previous significance and Y₁ is C₂-C₄-alkylene or hydroxypropylene; R₅₉, is C₁-C₄-alkyl or, together with R₆₀ and the nitrogen to which they are each attached, R₅₉ forms a pyrrolidine, piperidine, hexamethyleneimine or morpholine ring; R₆₀ is C₁-C₄-alkyl or, together with R₅₉ and the nitrogen to which they are each attached, R₆₀ forms a pyrrolidine, piperidine, hexamethyleneimine or morpholine ring; R₆₁ is hydrogen, C₁-C₄-alkyl, C₃-C₄-alkenyl, C₁-C₄-alkoxycarbonylmethyl, benzyl, C₂-C₄-hydroxyalkyl, C₂-C₄-cyanoalkyl or, together with R₅₉ and R₆₀ and the nitrogen atom to which they are each attached, R₆₁ forms a pyrrolidine, piperidine, hexamethyleneimine or morpholine ring; p is 0 or 1; and An(-) is an anion of an organic or inorganic acid; or,
a bistyrylphenyl fluorescent whitening agent of formula: in which R₅₅, Y₁, p and q have their previous significance and An(-) is an anion of an organic or inorganic acid; and R₆₂ and R₆₃, independently, are C₁-C₄-alkyl or C₂-C₃-alkenyl or R₆₂ and R₆₃, together with the nitrogen atom to which they are attached, form a pyrrolidine, piperidine, hexamethyleneimine or morpholine ring; R₆₄ is hydrogen, C₁-C₄-alkyl or C₂-C₃-alkenyl or R₆₂, R₆₃ and R₆₄, together with the nitrogen atom to which they are attached, form a pyridine or picoline ring; and Z is sulfur, -SO₂-, -SO₂NH-, -O-C₁-C₄-alkylene-COO- or -OCO-, or, in which the cationic bistyrylphenyl fluorescent whitening agent has the formula: in which R₅₅, R₆₂, R₆₃, R₆₄, Y₁, p and q have their previous significance and An(-) is an anion of an organic or inorganic acid; or, a amphoteric styrene fluorescent whitening agent offormula: in which R₅₅, R₆₂, R₆₃, Y₁ and q have their previous significance and Z, is oxygen, sulfur, a direct bond, -COO-, -CON(R₆₅)- or -SO₂N(R₆₅)- in which R₆₅ is hydrogen, C₁-C₄-alkyl or cyanoethyl and Q is -COO-or -SO₃, and,
in which the amine oxide fluorescent whitening agent has the formula: in which q has its previous significance and B is a brightener radical selected from a 4,4'-distyrylbiphenyl, 4,4'-divinyl-stilbene, and a 1,4'-distyrylbenzene, each optionally substituted by one to four substituents selected from halogen, C₁-C₄-alkyl, C₁-C₄-hydroxyalkyl, C₁-C₄-halogenoalkyl, C₁-C₄-cyanoalkyl, C₁-C₄-alkoxy- C₁-C₄-alkyl, phenyl- C₁-C₄-alkyl, carboxy- C₁-C₄-alkyl, carb- C₁-C₄-alkoxy-C₁-C₄-alkyl, C₁-C₄-alkenyl, C₅-C₈-cycloalkyl, C₁-C₄-alkoxy, C₁-C₄-alkenoxy, C₁-C₄-alkoxycarbonyl, carbamoyl, cyano, C₁-C₄-alkyl-sulfonyl, phenylsulfonyl, C₁-C₄-alkoxysulfonyl, sulfamoyl, hydroxyl, carboxyl, sulfo and trifluoromethyl;Z₂ is a direct bond between B and Y₂, an oxygen atom, a sulfur atom, -SO₂-,-SO₂-O-, -COO-, -CON(R₆₈)- or -SO₂N(R₆₈)- in which R₆₈ is hydrogen or C₁-C₄-alkyl optionally substituted by halogen, cyano, hydroxyl, C₂-C₅-carbalkoxy, C₁-C₄-alkoxy, phenyl, chlorophenyl, methylphenyl, methoxyphenyl, carbamoyl or sulfamoyl; Y₂ is C₂-C₄-alkylene or C₂-C₄-alkyleneoxy-C₂-C₄-alkylene, each optionally substituted by halogen, hydroxyl, C₂-C₅-carbalkoxy, C₁-C₄-alkoxy, phenyl, chlorophenyl, methylphenyl, methoxyphenyl, carbamoyl or sulfamoyl; and R₆₆ and R₆₇, independently, are C₅-C₈-cycloalkyl, C₁-C₄-alkyl or phenyl, each optionally substituted by halogen, hydroxyl, C₂-C₅-carbalkoxy, C₁-C₄-alkoxy, phenyl, chlorophenyl, methylphenyl, methoxyphenyl, carbamoyl or sulfamoyl; in which, in all the carbamoyl or sulfamoyl groups, the nitrogen atom is optionally substituted by one or two C₁-C₄-alkyl, C₁-C₄-hydroxyalkyl, C₂-C₅-cyanoalkyl, C₁-C₄-halogenoalkyl, benzyl or phenyl groups, or, a cationic fluorescent whitening agent of formula: in which q and Y₂ have their previous significance, and B₁ is a brightener radical; Z₃ is a direct bond, -SO₂-C₂-C₄-alkyleneoxy, -SO₂-C₂-C₄-alkylene-COO-, -SO₂-, -COO-, -SO₂-C₂-C₄-alkylene-CON(R₇₅)-or -SO₂N(R₇₅)- in which R₇₅ is hydrogen or C₁-C₄-alkyl optionally substituted by hydroxyl, halogen or cyano; R₇₀ is C₁-C₄-alkyl or C₂-C₄-alkenyl, each optionally substituted by halogen, cyano, hydroxy, C₁-C₄-alkoxycarbonyl or C₁-C₄-alkylcarbonyloxy, or R₇₀ is benzyl, optionally substituted by halogen, C₁-C₄-alkyl or C₁-C₄-alkoxy, or R₇₀, together with R₇₁ or Z₃, forms a pyrrolidine, piperidine or morpholine radical;R₇₁ is C₁-C₄-alkyl or C₂-C₄-alkenyl, each optionally substituted by halogen, cyano, hydroxy, C₁-C₄-alkoxycarbonyl or C₁-C₄-:alkylcarbonyloxy, or R₇₁ is benzyl, optionally substituted by halogen , C₁-C₄-alkyl or C₁-C₄-alkoxy, or R₇₁, together with R₇₀, forms a pyrrolidine, piperidine or morpholine radical; R₇₂ is C₁-C₄-alkyl; R₇₃ is hydrogen or
C₁-C₄-alkyl, optionally substituted by cyano, hydroxy, C₁-C₄-alkoxycarbonyl or C₁-C₄-alkylcarbonyloxy; and R₇₄ is C₁-C₄-alkyl or,
wherein said fluorescent whitening agent is a bis(triazinyl)diaminostilbene anionic fluorescent whitening agent of formula: or a dibenzofumylbiphenyl anionic fluorescent whitening agent of formula: and
or an anionic bistyrylphenyl fluorescent of formula: in which R₇₆ is phenyl optionally substituted by one or two SO₃M groups and R₇₇ is NH- C₁-C₄-alkyl, N(C₁-C₄-alkyl)₂, NH- C₁-C₄-alkoxy, N(C₁-C₄-alkoxy)₂, N(C₁₋C₄-alkyl)( C₁-C₄-hydroxyalkyl), N(C₁-C₄-hydroxyalkyl)₂; R₇₀ is H, C₁-C₄-alkyl, CN, CI or SO₃M; R₇₉ and R₈₀, independently, are H, C₁-C₄-alkyl, SO₃M, CN, CI or O- C₁-C₄-alkyl, provided that at least two of R₇₈, R₇₉ and R₈₀ are SO3M and the third group has solubilising character; R₈₁ is H, SO₃M, O- C₁-C₄-alkyl, CN, CI, COO- C₁-C₄-alkyl, or CON(C₁-C₄-alkyl)₂; and r is 0 or 1, and M has its previous significance.

The textile fibre material treated according to the use of the present invention may be composed of a wide variety of natural or synthetic fibres, e.g., wool, polyamide, cotton, polyester, polyacrylic, silk, polypropylene or mixtures thereof, preferably cotton.

The textile fibre material may be in the form of endless filaments (stretched or unstretched), staple fibres, flocks, hanks, textile filament yams, threads, nonwovens, felts, waddings, flocked structures or woven textile or bonded textile fabrics or knitted fabrics.

The amount of fluorescent whitening agent present in the composition used according to the use of the present invention may vary within a wide range, e.g. from 0.005 to 20 %, based on the weight of the textile fibre material, depending on the particular composition used in the used of the present invention. Thus, when the composition is an aqueous textile finishing composition, the amount of fluorescent whitening agent present in the composition preferably ranges from 0.01 to 3%, especially from 0.05 to 1%, based on the weight of the textile fibre material. When the composition is a detergent composition, the amount of fluorescent whitening agent present in the composition preferably ranges from 0.005 to 2%, especially from 0.01 to 1%, based on the weight of the textile fibre material. When the composition is a post-wash fabric care composition, the amount of fluorescent whitening agent present in the composition preferably ranges from 0.1 to 20%, especially from 1 to 10%, based on the weight of the textile fibre material.

With particular reference to the use of a fluorescent whitening agent in a composition which is an aqueous textile finishing composition, preferred 4,4'-bis-(triazinylamino)-stilbene-2,2'-disulfonic acids are those having the formula: in which R₁ and R₂, independently, are phenyl, mono- or disulfonated phenyl, phenylamino, mono- or disulfonated phenylamino, morpholino, N(CH₂CH₂OH)₂, -N(CH₃)(CH₂CH₂OH), -NH₂, -N(C₁-C₄alkyl)₂, -OCH₃, -Cl, -NH-CH₂CH₂SO₃H or NH-CH₂CH₂OH; and M is H, Na, K, Ca, Mg, ammonium, mono-, di-, tri- or tetra- C₁-C₄-alkylammonium, mono-, di- or tri- C₁-C₄-hydroayalkylarnmonium or ammonium that is di- or tri-substituted with by a mixture of C₁-C₄-alkyl and C₁-C₄-hydroxyalkyl groups.

Especially preferred compounds of formula (1) are those in which each R₁ is 2,5-disulfophenyl and each R₂ is morpholino; or each R₁ is 2,5-disulfophenyl and each R₂ is N(CH₂CH₂); or each R₁ is 3-sulfophenyl and each R₂ is NH(CH₂CH₂OH) or N(CH₂CH₂OH)₂; or each R₁ is 4-sulfophenyl and each R₂ is N(CH₂CH₂OH)₂; and, in each case, the sulfo group is SO₃M in which M is sodium.

Preferred 4,4'-bis-(triazol-2-yl)stilbene-2,2'-disulfonic acids are those having the formula: in which R₃ and R₄, independently, are H, C₁-C₄-alkyl, phenyl or monosulfonated phenyl; and M has its previous significance.

Especially preferred compounds of formula (2) are those in which R₃ is phenyl, R₄ is H and M is sodium.

One preferred 4,4'-(diphenyl)-stilbene is that having the formula:

Preferably, 4,4'-distyryl-biphenyls used are those of formula: in which R₅ and R₆, independently, are H, SO₃M, SO₂N(C₁-C₄-alkyl)₂, O-(C₁-C₄-alkyl), CN, Cl, COO(C₁-C₄-alkyl), CON(C₁-C₄-alkyl)₂ or O(CH₂)₃N^{⊕}(CH₃)₂An^{⊖} in which An^{⊖} is an anion of an organic or inorganic acid, in particular a formate, acetate, propionate, glycolate, lactate, acrylate, methanephosphonate, phosphite, dimethyl or diethyl phosphite anion , or a mixture thereof; and n is 0 or 1.

Especially preferred compounds of formula (4) are those in which n is 1 and each R₅ is a 2-SO₃M group in which M is sodium and each R₆ is H, or each R₅ is O(CH₂)₃N^{⊕}(CH₃)₂An^{⊖} in which An^{⊖} is acetate.

Preferred 4-phenyl-4'-benzoxazolyl-stilbenes have the formula: in which R₇ and R₈, independently, are H, Cl, C₁-C₄-alkyl or SO₂-C₁-C₄-alkyl.

An especially preferred compound of formulae (5) is that in which R₇ is 4-CH₃ and R₈ is 2-CH₃.

Preferably, stilbenyl-naphthotriazoles used are those of formula: in which R₉ is H or Cl; R₁₀ is SO₃M, SO₂N(C₁-C₄-alkyl)₂, SO₂O-phenyl or CN; R₁₁ is H or SO₃M; and M has its previous significance.

Especially preferred compounds of formula (6) are those in which R₉ and R₁₁ are H and R₁₀ is 2-SO₃M in which M is Na.

Preferably, 4-styryl-stilbenes used are those of formula: in which R₁₂ and R₁₃, independently, are H, SO₃M, SO₂N(C₁-C₄-alkyl)₂, O-(C₁-C₄-alkyl), CN, Cl, COO(C₁-C₄-alkyl), CON(C₁-C₄-alkyl)₂ or O(CH₂)₃N^{⊕}(CH₃)₂An^{⊖} in which An^{⊖} is an anion of an organic or inorganic acid, in particular a formate, acetate, propionate, glcolate, lactate, acrylate, methanephosphonate, phosphite, dimethyl or diethyl phosphite anion, or a mixture thereof.

Especially preferred compounds of formula (7) are those in which each of R₁₂ and R₁₃ is 2-cyano, 2-SO₃M in which M is sodium or O(CH₂)₃N^{⊕}(CH₃)₂An^{⊖} in which An^{⊖} is acetate.

Preferred bis-(benzoxazol-2-yl) derivatives are those of formula: in which R₁₄, independently, is H, C(CH₃)₃, C(CH₃)₂-phenyl, C₁-C₄-alkyl or COO-C₁-C₄-alkyl, and X is -CH=CH- or a group of formula: Especially preferred compounds of formula (8) are those in which each R₁₄ is H and X is or one group R₁₄ in each ring is 2-methyl and the other R₁₄ is H and X is -CH=CH-; or one group R₁₄ in each ring is 2-C(CH₃)₃ and the other R₁₄ is H and X is

Preferred bis-(benzimidazol-2-yl) derivatives are those of formula: in which R₁₅ and R₁₆, independently, are H, C₁-C₄-alkyl or CH₂CH₂OH; R₁₇ is H or SO₃M; X₁ is -CH=CH- or a group of formula: and M has its previous significance.

Especially preferred compounds of formula (9) are those in which R₁₅ and R₁₆ are each H, R₁₇ is SO₃M in which M is sodium and X₁ is -CH=CH-.

Preferred coumarines are those of formula: in which R₁₈ is H, Cl or CH₂COOH, R₁₉ is H, phenyl, COO-C₁-C₄-alkyl or a group formula: and R₂₀ is O-C₁-C₄-alkyl, N(C₁-C₄-alkyl)₂, NH-CO-C₁-C₄-alkyl or a group of formula: or in which R₁, R₂, R₃ and R₄ have their previous significance and R₂₁ is H, C₁-C₄-alkyl or phenyl.

Especially preferred compounds of formula (10) are those having the formula: or

Preferably, pyrazolines used are those having the formula: in which R₂₂ is H, CI or N(C₁-C₄-alkyl)₂, R₂₃ is H, Cl, SO₃M, SO₂NH₂, SO₂NH-(C₁-C₄-alkyl), COO-C₁-C₄-alkyl, SO₂-C₁-C₄-alkyl, SO₂NHCH₂CH₂CH₂N^{⊕}(CH₃)₃ or SO₂CH₂CH₂N^{⊕}H(C₁-C₄-alkyl)₂ An^{⊖}, R₂₄ and R₂₅ are the same or different and each is H, C₁-C₄-alkyl or phenyl and R₂₆ is H or Cl; and An^{⊖} and M have their previous significance.

Especially preferred compounds of formula (13) are those in which R₂₂ is Cl, R₂₃ is SO₂CH₂CH₂N^{⊕}H(C₁-C₄-alkyl)₂ An^{⊖} in which An^{⊖} is phosphite and R₂₄, R₂₅ and R₂₆ are each H; or those those having the formula: or

Preferred naphthalimides are those of formula: in which R₂₇ is C₁-C₄-alkyl or CH₂CH₂CH₂N^{⊕}(CH₃)₃; R₂₈ and R₂₉, independently, are O-C₁-C₄-alkyl, SO₃M or NH-CO-C₁-C₄-alkyl; and M has its previous significance.

Especially preferred compounds of formula (16) are those having the formula:

Preferred triazinyl-pyrenes used are those of formula: in which each R₃₀, independently, is C₁-C₄-alkoxy.

Especially preferred compounds of formula (19) are those in which each R₃₀ is methoxy.

Preferred 2-styryl-benzoxazole- or -naphthoxazole derivatives are those having the formula: in which R₃₁ is CN, Cl, COO-C₁-C₄-alkyl or phenyl; R₃₂ and R₃₃ are the atoms required to form a fused benzene ring or R₃₃ and R₃₅, independently, are H or C₁-C₄-alkyl; and R₃₄ is H, C₁-C₄-alkyl or phenyl.

Especially preferred compounds of formula (20) are those in which R₃₁ is a 4-phenyl group and each of R₃₂ to R₃₅ is H.

Preferred benzimidazole-benzofuran derivatives are those having the formula: in which R₃₆ is C₁-C₄-alkoxy; R₃₇ and R₃₈, independently, are C₁-C₄-alkyl; and An^{⊖} has its previous significance.

A particularly preferred compound of formula (21) is that in which R₃₆ is methoxy, R₃₇ and R₃₈ are each methyl and An(-) is methane sulfonate.

Preferred oxanilide derivatives include those having the formula: in which R₃₉ is C₁-C₄alkoxy, R₄₁ is C₁-C₄alkyl, C₁-C₄alkyl-SO₃M or C₁-C₄alkoxy-SO₃M in which M has its previous significance and R₄₀ and R₄₂ are the same and each is hydrogen, tert. butyl or SO₃M in which M has its previous significance.

When a fluorescent whitening agent is used in a composition which is a textile finishing bath, the fluorescent whitening agent may be in various formulations such as:
a) in mixtures with dyes (shading) or pigments, especially white pigments;
b) in mixtures with carriers, wetting agents, antioxidants, e.g., sterically hindered amines, UV absorbers and/or chemical bleaching agents; or
c) in admixture with crosslinking or finishing agents (such as starch or synthetic finishes), and in combination with a wide variety of textile finishing processes, especially synthetic resin finishes, e.g. creaseproof finishes (wash-and-wear, permanent press or non-iron), as well as flameproof finishes, soft handle finishes, antisoiling finishes, antistatic finishes or antimicrobial finishes.

With refernce to the use of a fluorescent whitening agent in a detergent composition the C₁-C₄-alkyl groups of compounds of formulae (23) to (30) are, e.g., methyl, ethyl, n-propyl, isopropyl and n-butyl, especially methyl. Aryl groups are naphthyl or, especially, phenyl.

It will be appreciated that the protection afforded to the wearer of the textile material, washed according to this detergent composition aspect of the use of the invention, will last longer when a fluorescent whitening agent is used which has a high lightfastness.

Furthermore, preferred fluorescent whitening agents for use in the present invention have a spectrum covering a relatively low wavelength range, that is exhibiting rather reddish shades. Examples of such fluorescent whitening agents include compounds of formula (23) in which R₄₃ and R₄₄are each non-aromatic substituents. such as compounds of formula (23) in which R₄₃ and R₄₄, independendy, are NH-C₁-C₄-alkyl, O-C₁-C₄-alkyl or morpholino; as well as compounds of formula (26) in which n is 1.

Preferred compounds of formula (23) are those in which R₄₃ and R₄₄, independently, are O-methyl, O-phenyl, NH₂, NH-methyl, N(methyl)₂, N(methyl)(hydroxyethyl), NH-ethyl, N(hydroxyethyl)₂, NH-phenyl, S-methyl(phenyl), Cl or OH.

Specific examples of preferred compounds of formula (23) are those having the formulae:

Specific preferred examples of compounds of formula (24) are those of formulae: in which n has its previous significance.

Preferred examples of compounds of formula (26) are those having the formulae:

Preferred examples of compounds of formula (27) are those of formulae:

A preferred example of a compound of formula (30) is that having the formula:

The compounds of formulae (23) to (30) are known and may be obtained by known methods.

In the post-wash care compositions comprising compound (48) An(-) has its previous significance and is preferably the chloride, bromide, iodide, methosulfate, ethosulfate, benzenesulfonate or p-toluenesulfonate anion when R₅₈ is C₁-C₄-alkyl or An(-) is preferably the formate, acetate, propionate or benzoate anion when R₅₈ is beta -hydroxy- gamma -chloropropyl, beta -cyanoethyl or C₁-C₄-alkoxy-carbonylethyl.

Preferred compounds of formula (48) are those in which Y is 1,4-phenylene or 4,4'-diphenylene; R₅₅ is hydrogen, methyl or cyano; R₅₆ and R₅₇ are each methyl or cyano; and R₅₈ and An(-) have their previously indicated preferred meanings.

One particularly preferred compound of formula (48) is that having the formula: The compounds of formula (48) and their production are described in US-A-4 009 193.

Preferred compounds of formula (50) are those in which q is 1; R₅₅ is hydrogen, chlorine, C₁-C₄-alkyl or C₁-C₄-alkoxy; Y₁ is (CH₂)₂; R₅₉ and R₆₀ are the same and each is methyl or ethyl; R₆₁ is methyl or ethyl; p is 1; and An(-) is CH₃OSO₃ or C₂H₅OSO₃.

The compounds of formula (50) and their production are described in US-A-4 339 393.

Preferred cationic bistyrylphenyl fluorescent whitening agents of formula (51) are those in which R₅₅ is hydrogen, chlorine, C₁-C₄-alkyl or C₁-C₄-alkoxy; R₆₂ and R₆₃, independently, are C₁-C₄-alkyl or, together with the nitrogen atom to which they are attached, form a pyrrolidine, piperidine or morpholine ring; R₆₄ is hydrogen, C₁-C₄-alkyl or C₃-C₄-alkenyl or R₆₂, R₆₃ and R₆₄, together with the nitrogen atom to which they are attached, form a pyridine ring; and Z is sulfur, -SO₂-or -SO₂NH-.

The compounds of formula (51) and their production are described in US-A-4 486 352.

Preferred compounds of formula (52) are those in which q is 1; R₅₅ is hydrogen, chlorine, C₁-C₄-alkyl or C₁-C₄-alkoxy; R₆₂ and R₆₃, independently, are C₁-C₄-alkyl or, together with the nitrogen atom to which they are attached, form a pyrrolidine, piperidine or morpholine ring; R₆₄ is hydrogen, C₁-C₄-alkyl or C₃-C₄-alkenyl or R₆₂, R₆₃ and R₆₄, together with the nitrogen atom to which they are attached, form a pyridine ring.

The compounds of formula (52) and their production are described in US-A-4 602 087.

Preferred compounds of formula (53) are those in which Z, is oxygen, a direct bond, -CONH-, -SO₂NH or -COO-, especially oxygen; q is 1; R₆₂ is hydrogen, C₁-C₄-alkyl, methoxy or chlorine; and R₆₃, R₆₄, Y₁ and Q have their previous significance.

The compounds of formula (53) and their production are described in US-A-4 478 598.

Preferred is compound of formula (53), in which the brightener radicals B are those having the formula: in which q has its previous significance and the rings are optionally substituted as indicated above.

Preferably Z₂ is oxygen, -SO₂- or -SO₂N(R₆₉)- in which R₆₉ is hydrogen or C₁-C₄-alkyl optionally substituted by hydroxyl, halogen or cyano; and R₆₆ and R₆₇, independently, are C₁-C₄-alkyl optionally substituted by halogen, cyano, hydroxyl, C₁-C₄-alkoxy, phenyl, chlorophenyl, methylphenyl, methoxyphenyl or C₂-C₅-alkoxycarbonyl. Other preferred compounds of formula (52) are those in which Z₂ is oxygen, sulfur, -SO₂-, -CON(R₆₉)- or -SO₂N(R₆₉)- in which R₆₉ is hydrogen or C₁-C₄-alkyl optionally substituted by hydroxyl, halogen or cyano; and Y₂ is C₁-C₄-alkylene.

The compounds of formula (54) and their production are described in US-A-4 539 161.

Preferably, brightener radical B₁ has the formula: or the formula: each optionally substituted by one to four substituents selected from halogen, C₁-C₄-alkyl, C₁-C₄-hydroxyalkyl, C₁-C₄-halogenoalkyl, C₁-C₄-cyanoalkyl, C₁-C₄-alkoxy-C₁-C₄-alkyl, phenyl- C₁-C₄-alkyl, carboxy- C₁-C₄-alkyl, carb-C₁-C₄-alkoxy-C₁-C₄-alkyl, C₁-C₄-alkenyl, C₅-C₈-cyaoalkyl, C₁-C₄-alkoxy, C₁-C₄-alkenoxy, C₁-C₄-alkoxycarbonyl, carbamoyl, cyano, C₁-C₄-alkyl-sulfonyl, phenylsulfonyl, C₁-C₄-alkoxysulfonyl, sulfamoyl, hydroxyl, carboxyl, sulfo and trifluoromethyl.

The compounds of formula (55) and their production are described in GB-A-2 023 605.

In the compounds of formulae (56) to (58), C₁-C₄-alkyl groups are, e.g., methyl, ethyl, n-propyl, isopropyl and n-butyl, especially methyl. Aryl groups are naphthyl or, especially, phenyl.

Specific examples of preferred compounds of formula (56) are those having the formula (31), (32) or (34), each as hereinbefore defined.

Preferred examples of compounds of formula (57) are those of formula (43), (44), (45) or (46), each as hereinbefore defined.

Preferred examples of compounds of formula (58) are those having the formula (40), (41) or (42), each as hereinbefore defined.

The compounds of formulae (56) to (58) are known and may be obtained by known methods.

With respect to that aspect of the use of the present invention in which the fluorescent whitening agent is applied from a textile finishing composition, of particular interest is the co-use of the fluorescent whitening agent with a UV absorber.

The UV absorber used may be any of the wide range of known UV absorbers, that is organic compounds which readily absorb UV light, especially in the range lambda =280 to 400 nm, and which convert the absorbed energy, by a chemical intermediate reaction, into non-interfering, stable compounds or into non-interfering forms of energy. If the textile finishing composition is used in combination with a rinse cycle fabric softener composition, the absorber used should, of course, be compatible with the rinse cycle fabric softener composition. In such instances, preferably, the UV absorber used is one which is capable of being absorbed on to the washed textile article during a rinse cycle fabric softener treatment.

The UV absorber used may be, e.g., an oxalic anilide, an o-hydroxybenzophenone, an o-hydroxyaryl-1,3,5-triazine, a sulphonated-1,3,5-triazine, an o-hydroxyphenylbenzotriazole, a 2-aryl-2H-benzotriazole, a salicylic acid ester, a substituted acrylonitrile, a substituted arylaminoethylene or a nitrilohydrazone.

Such known UV absorbers for use in the: present invention are described, for example, in the US patent specifications 2 777 828, 2 853 521, 3 118 887, 3 259 627, 3 293 247, 3 382 183,3 403 183, 3 423 360, 4 127 586, 4 141903, 4 230 867, 4 675 352 and 4 698 064.

Preferred UV absorbers for use in the present invention include those of the benzo-triazine or benzo-triazole class.

One preferred class of benzo-triazine UV absorbers is that having the formula: in which R₈₂ and R₈₃, independently, are hydrogen, hydroxy or C₁-C₅alkoxy.

A second preferred class of triazine UV absorbers is that having the formula: in which at least one of R₈₄, R₈₅ and R₈₆ is a radical of formula: in which M has its previous significance; m is 1 or 2; and the remaining substituent(s) R₈₄, R₈₅ and R₈₆ are, independently, amino, C₁-C₁₂alkyl, C₁-C₁₂alkoxy, C₁-C₁₂alkylthio, mono- or di-C₁-C₁₂alkylamino, phenyl, phenylthio, anilino or
N-phenyl-N-C₁-C₄alkylamino, preferably N-phenyl-N-methylamino or
N-phenyl-N-ethylamino, the respective phenyl substituents being optionally substituted by C₁-C₁₂alkyl or -alkoxy, C₅-C₈cycloalkyl or halogen.

A third preferred class of triazine UV absorbers is that having the formula: in which R₈₇ is hydrogen or hydroxy; R₈₈, independently, are hydrogen or C₁-C₄alkyl; n₁ is 1 or 2; and B is a group of formula: in which n₂ is an integer from 2 to 6 and is preferably 2 or 3; Y₃ and Y₄, independently, are C₁-C₄alkyl optionally substituted by halogen, cyano, hydroxy or C₁-C₄alkoxy or Y₃ and Y₄, together with the nitrogen atom to which they are each attached, form a 5-7 membered heterocyclic ring, preferably a morpholine, pyrrolidine, piperidine or hexamethyleneimine ring; Y₅ is hydrogen, C₃-C₄alkenyl or C₁-C₄alkyl optionally substituted by cyano, hydroxy or C₁-C₄alkoxy or Y₃, Y₄ and Y₅, together with the nitrogen atom to which they are each attached, form a pyridine or picoline ring; and X₁^{⊖} is a colourless anion, preferably CH₃OSO₃^{⊖} or C₂H₅OSO₃^{⊖}.

One preferred class of triazole UV absorbers is that having the formula: in which T₁ is chlorine or, preferably, hydrogen; and T₂ is a random statistical mixture of at least three isomeric branched sec. C₈-C₃₀, preferably C₈₋C₁₆, especially C₉-C₁₂alkyl groups, each having the formula -CH(E₁)(E₂) in which E₁ is a straight chain C₁-C₄alkyl group and E₂ is a straight chain C₄-C₁₅alkyl group, the total number of carbon atoms in E₁ and E₂ being from 7 to 29.

A second preferred class of triazole UV absorbers is that having the formula: in which M has its previous significance, but is preferably sodium, and T₃ is hydrogen, C₁-C₁₂alkyl or benzyl.

A third preferred class of triazole UV absorbers is that having the formula: in which B has its previous significance.

In the compounds of formulae (59) to (65), C₁-C₁₂alkyl groups R₈₄, R₈₅, R₈₆ and T₃ may be methyl, ethyl, n-propyl, isopropyl, n-butyl, isobutyl, tert.-butyl,n-amyl, n-hexyl, n-heptyl, n-octyl, isooctyl, n-nonyl, n-decyl, n-undecyl and n-dodecyl, methyl and ethyl being preferred, except in the case of T₃ for which isobutyl is preferred. C₈-C₃₀alkyl groups T₂ include sec.octyl, decyl, dodecyl, tridecyl, tetradecyl, hexadecyl, octadecyl, eicosyl and triacontyl groups.

C₁-C₅Alkoxy groups R₈₂ or R₈₃ may be, e.g., methoxy, ethoxy, n-propoxy, isopropoxy, n-butoxy, isobutoxy, tert.-butoxy or n-amyloxy, preferably methoxy or ethoxy, especially methoxy. C₁-C₁₂Alkoxy groups R₈₄, R₈₅ and R₈₆ include those indicated for the C₁-C₅alkoxy groups R₈₂ or R₈₃ together with, e.g., n-hexoxy, n-heptoxy, n-octoxy, isooctoxy, n-nonoxy, n-decoxy, n-undecoxy and n-dodecoxy, methoxy and ethoxy being preferred.

C₁-C₁₂Alkylthio groups R₈₄, R₈₅ and R₈₆ may be, e.g., methylthio, ethylthio, n-propylthio, isopropylthio, n-butylthio, isobutylthio, tert.-butylthio, n-amylthio, hexylthio, n-heptylthio, n-octylthio, isooctylthio, n-nonylthio, n-decylthio, n-undecylthio and n-dodecylthio, methylthio and ethylthio being preferred.

C₁-C₁₂Mono- or di-alkylamino groups R₈₄, R₈₅ and R₈₆ include, e.g., mono- or di-methylamino, ethylamino, n-propylamino, isopropylamino, n-butylamino, isobutylamino, tert.-butylamino, n-amylamino, n-hexylamino, n-heptylamino, n-octylamino, isooctylamino, n-nonylamino, n-decylamino, n-undecylamino and n-dodecylamino, mono- or di-methylamino or ethylamino being preferred.

The alkyl radicals in the mono-, di-, tri- or tetra-C₁-C₄alkylammonium groups M are preferably methyl. Mono-, di- or tri-C₁-C₄hydroxyalkylammonium groups M are preferably those derived from ethanolamine, di-ethanolamine or tri-ethanolamine. When M is ammonium that is di- or tri-substituted by a mixture of C₁-C₄alkyl and C₁-C₄hydroxyalkyl groups, it is preferably N-methyl-N-ethanolamine or N,N-dimethyl-N-ethanolamine. M is preferably, however, hydrogen or sodium.

Preferred compounds of formula (59) are those having the formulae:

The compounds of formula (59) are known and may be prepared e.g. by the method described in U.S. Patent 3 118 887.

Preferred compounds of formula (60) are those having the formula: in which R₈₉ and R₉₀, independently, are C₁-C₁₂alkyl, preferably methyl; m is 1 or 2; M₁ is hydrogen, sodium, potassium, calcium, magnesium, ammonium or tetra-C₁-C₁₂alkylammonium, preferably hydrogen; and n₃ and n₄, independently, are 0, 1 or 2, preferably 1 or 2.

Particularly preferred compounds of formula (73) are:
2,4-diphenyl-6-[2-hydroxy-4-(2-hydroxy-3-sulfopropoxy)-phenyl]-1,3,5-triazine;
2-phenyl-4,6-bis-[2-hydroxy-4-(2-hydroxy-3-sulfopropoxy)- phenyl] -1,3,5-triazine;
2,4-bis(2,4-dimethylphenyl)-6-[2-hydroxy-4-(2-hydroxy-3-sulfopropoxy)-phenyl] -1,3,5-triazine; and
2,4-bis(4-methylphenyl)-6-[2-hydroxy-4-(2-hydroxy-3-sulfo propoxy)-phenyl] -1,3,5-triazine.

The compounds of formula (60) are known and may be prepared in the manner, e.g., described in US Patent 5 197 991.

The compounds of formula (63) are known and may be prepared in the manner, e.g., described in US Patent 4 675 352.

The compounds of formula (64) are known and may be prepared in the manner, e.g., described in EP-A-0 314 620.

The compounds of formula (65) are known and may be prepared in the manner, e.g., described in EP-A-0 357 545.

The use of the present invention is advantageously conducted in an aqueous medium in which the relevant fluorescent whitening agent is present in solution or as a fine dispersion.

Although most are readily water-soluble, some of the fluorescent whitening agents or UV absorbers for use in the method according to the present invention may be only sparingly soluble in water and may need to be applied in dispersed or emulsified form. For this purpose, they may be milled with an appropriate dispersant, conveniently using quartz balls and an impeller, down to a particle size of 1-2 microns.

As dispersing agents for such sparingly-soluble compounds there may be mentioned:
acid esters or their salts of alkylene oxide adducts, e.g., acid esters or their salts of a polyadduct of 4 to 40 moles of ethylene oxide with 1 mole of a phenol, or phosphoric acid esters of the adduct of 6 to 30 moles of ethylene oxide with 1 mole of 4-nonylphenol, 1 mole of dinonylphenol or, especially, with 1 mole of compounds which have been produced by the addition of 1 to 3 moles of styrenes on to 1 mole of phenol;
polystyrene sulphonates;
fatty acid taurides;
alkylated diphenyloxide-mono- or -di-sulphonates;
sulphonates of polycarboxylic acid esters;
addition products of 1 to 60, preferably 2 to 30 moles of ethylene oxide and/or propylene oxide on to fatty amines, fatty amides, fatty acids or fatty alcohols, each having 8 to 22 carbon atoms, or on to tri- to hexavalent C3-C6alkanols, the addition products having been converted into an acid ester with an organic dicarboxylic acid or with an inorganic polybasic acid;
lignin sulphonates; and, in particular
formaldehyde condensation products, e.g., condensation products of lignin sulphonates and/or phenol and formaldehyde; condensation products of formaldehyde with aromatic sulphonic acids, e.g., condensation products of ditolylethersulphonates and formaldehyde; condensation products of naphthalenesulphonic acid and/or naphthol- or naphthylaminesulphonic acids and formaldehyde; condensation products of phenolsulphonic acids and/or sulphonated dihydroxydiphenylsulphone and phenols or cresols with formaldehyde and/or urea; or condensation products of diphenyloxidedisulphonic acid derivatives with formaldehyde.

With particular reference to that aspect of the method of the present invention which is effected from a textile finishing composition, and depending on the type of fluorescent whitening agent used, it may be beneficial to carry out the treatment in a neutral, alkaline or acidic bath. The method is usually conducted in the temperature range of from 20 to 140°C.,for example at or near to the boiling point of the aqueous bath, e.g. at about 90°C.

Solutions of the fluorescent whitening agent, or its emulsions in organic solvents may also be used in the method of the present invention. For example, the so-called solvent dyeing (pad thermofix application) or exhaust dyeing methods in dyeing machines may be used.

In certain cases, the fluorescent whitening agent is made fully effective by an after-treatment. This may comprise a chemical treatment such as treatment with an acid, a thermal treatment or a combined thermal/chemical treatment.

It is often advantageous to use the fluorescent whitening agent in admixture with an assistant or extender such as anhydrous sodium sulfate, sodium sulfate decahydrate, sodium chloride, sodium carbonate, an alkali metal phosphate such as sodium or potassium orthophosphate, sodium or potassium pyrophosphate or sodium or potassium tripolyphosphate, or an alkali metal silicate such as sodium silicate.

The preferred fluorescent whitening agent for use in the method according to the present invention will vary depending on the fibre from which the treated fabric is composed.

Thus, in relation to that aspect of the present invention in which the fluorescent whitening agent is applied from a textile finishing composition, there is preferably used, for the treatment of cotton fabrics, a fluorescent whitening agent of formula (1), (2), (4), (6) or (9) is preferably used; for polyester fabrics, a fluorescent whitening agent of formula (4), (5), (6), (7), (8), (10), (12), (19) or (20) is preferably used; for the treatment of polyamide, a fluorescent whitening agent of formula (1), (2), (4), (5), (6), (7), (8), (10), (11) or (20) is preferably used; for the treatment of polyacrylonitrile, a fluorescent whitening agent of formula (6), (9), (10), (11), (12) or (21) is preferably used; for wool or silk, a fluorescent whitening agent of formula (1), (2), (4), (6), (9), (10) or (11) is preferably used; and for polypropylene, a fluorescent whitening agent of formula (8) is preferably used.

In relation to that aspect of the present invention in which the fluorescent whitening agent is applied from a detergent composition, the use according to the present invention is preferably effected by washing the textile fibre material at least once with the detergent composition, preferably at a temperature ranging from 10 to 100°C., especially from 15 to 60°C.

The detergent composition used preferably comprises:
i) 5-90%, preferably 5-70% of an anionic surfactant and/or a nonionic surfactant;
ii) 5-70%, preferably 5-40% of a builder;
iii) 0-30%, preferably 1-12% of a peroxide;
iv) 0-10%, preferably 1-6% of a peroxide activator and/or 0-1%, preferably 0.1-3% of a bleaching catalyst;
v) 0.005-2%, preferably 0.01-1% of at least one fluorescent whitening agent which absorbs radiation in the wavelength range 280-400 nm; and
vi) 0.005-10%, preferably 0.1-5% of of one or more auxiliaries, each by weight, based on the total weight of the detergent.

The detergent may be formulated as a solid, as an aqueous liquid comprising 5-50, preferably 10-35% water or as a non-aqueous liquid detergent, containing not more than 5, preferably 0-1 wt.% of water, and based on a suspension of a builder in a non-ionic surfactant, as described, e.g., in GB-A-2158454.

The anionic surfactant component may be, e.g., a sulphate, sulphonate or carboxylate surfactant, or a mixture of these.

Preferred sulphates are alkyl sulphates having 12-22 carbon atoms in the alkyl radical, optionally in combination with alkyl ethoxy sulphates having 10-20 carbon atoms in the alkyl radical.

Preferred sulphonates include alkyl benzene sulphonates having 9-15 carbon atoms in the alkyl radical.

In each case, the cation is preferably an alkali metal, especially sodium.

Preferred carboxylates are alkali metal sarcosinates of formula R-CO(R¹)CH₂COOM¹ in which R is alkyl or alkenyl having 9-17 carbon atoms in the alkyl or alkenyl radical, R¹ is C₁-C₄ alkyl and M¹ is alkali metal.

The nonionic surfactant component may be, e.g., a condensate of ethylene oxide with a C₉-C₁₅ primary alcohol having 3-8 moles of ethylene oxide per mole.

The builder component may be an alkali metal phosphate, especially a tripolyphosphate; a carbonate or bicarbonate, especially the sodium salts thereof; a silicate; an aluminosilicate; a polycarboxylate; a polycarboxylic acid; an organic phosphonate; or an aminoalkylene poly (alkylene phosphonate); or a mixture of these.

Preferred silicates are crystalline layered sodium silicates of the formula NaHSiₘO_{2m+1·}pH₂O or Na₂SiₘO_{2m+1·}pH₂O in which m is a number from 1.9 to 4 and p is 0 to 20.

Preferred aluminosilicates are the commercially-available synthetic materials designated as Zeolites A, B, X, and HS, or mixtures of these. Zeolite A is preferred.

Preferred polycarboxylates include hydroxypolycarboxylates, in particular citrates, polyacrylates and their copolymers with maleic anhydride.

Preferred polycarboxylic acids include nitrilotriacetic acid and ethylene diamine tetra-acetic acid.

Preferred organic phosphonates or aminoalkylene poly (alkylene phosphonates) are alkali metal ethane 1-hydroxy diphosphonates, nitrilo trimethylene phosphonates, ethylene diamine tetra methylene phosphonates and diethylene triamine penta methylene phosphonates.

Any peroxide component may be any organic or inorganic peroxide compound, described in the literature or available on the market, which bleaches textiles at conventional washing temperatures, e.g. temperatures in the range of from 5°C. to 90°C. In particular, the organic peroxides are, for example, monoperoxides or polyperoxides having alkyl chains of at least 3, preferably 6 to 20, carbon atoms; in particular diperoxydicarboxylates having 6 to 12 C atoms, such as diperoxyperazelates, diperoxypersebacates, diperoxyphthalates and/or diperoxydodecanedioates, especially their corresponding free acids, are of interest. It is preferred, however, to employ very active inorganic peroxides, such as persulphate, perborate and/or percarbonate. It is, of course, also possible to employ mixtures of organic and/or inorganic peroxides. The peroxides, especially the inorganic peroxides, are preferably activated by the inclusion of an activator such as tetraacetyl ethylenediamine or nonoyloxybenzene sulfonate. Bleaching catalysts which may be added include, e.g., enzymatic peroxide precursors and/or metal complexes. Preferred metal complexes are manganese or iron complexes such as manganese or iron phthalocyanines or the complexes described in EP-A-0 509 787.

The detergents used will usually contain one or more auxiliaries such as soil suspending agents, for example sodium carboxymethylcellulose; salts for adjusting the pH, for example alkali or alkaline earth metal silicates; foam regulators, for example soap; salts for adjusting the spray drying and granulating properties, for example sodium sulphate; perfumes; and also, if appropriate, antistatic and softening agents; such as smectite clays; enzymes, such as amylases; photobleaching agents; pigments; and/or shading agents. These constituents should, of course, be stable to any bleaching system employed.

The preferred fluorescent whitening agent for use in the detergent used according to the present invention will vary depending on the fibre from which the treated fabric is composed.

Thus, for the treatment of polyester fabrics from a detergent composition, a fluorescent whitening agent of formula (28) is preferably used. For the treatment of polyamide, a fluorescent whitening agent of formula (29), (30) or (34) is preferably used. For wool, a fluorescent whitening agent of formula (29), (30) or (37) is preferably used

Relative to the use of a conventional UV absorber, the use in the present invention of a fluorescent whitening agent which absorbs radiation in the wavelength range 280-400 nm from a detergent composition has the following advantages: easier application since it exhausts on to the fibre; coloured textile goods can be washed with a detergent composition according to the claimed use (previously it was generally believed that FWAs had no useful role to play in detergents for coloured goods - see, e.g., A.E.Lee "Technology developments in laundry products", Proc. of the 3^{rd} World Conference on Detergents, Montreux, Sept. 1994, AOCS Press, p.73, § "Color variants"); the UV protection is regularly renewed on washing; yellowing of the textile material caused by o-hydroxy groups in the UV absorber is avoided; minor amounts of the fluorescent whitening agent provide very high extinction values; the textile material is more wash resistant; and higher SPF values are attainable.

With respect to that aspect of the method of the present invention in which the fluorescent whitening agent is applied to the textile fibre material via a post-wash fabric care composition, the present invention provides, as a further aspect, a stable, concentrated fabric care composition comprising 0.3 to 10, preferably 0.3 to 3% by weight of a fluorescent whitening agent which is compatible with a fabric care ingredient, preferably a cationic, amphoteric or anionic fluorescent whitening agent, based on the total weight of the composition, and a fabric care ingredient, preferably a fabric softener, a stain release or stain repellant ingredient or a water-proofing agent, the remainder being substantially water.

The fabric care ingredient is preferably present in an amount of from 2 to 25, preferably 5 to 20% by weight, based on the total weight of the composition.

Preferred examples of cationic fabric softening agents include imidazolines, quaternary ammonium compounds, ester amide amine salts, as well as mixtures thereof.

Preferred imidazoline cationic fabric softening agents are those having the formula: in which R₉₁ is hydrogen or C₁-C₄alkyl; R₉₂ is a C₈-C₃₀aliphatic residue; R₉₃ is -C₂H₄-O(C=O)-R₉₂ or -C₂H₄-NH(C=O)-R₉₂; and An(-) has its previous significance.

Preferably R₉₁ is hydrogen or methyl; R₉₂ is C₁₄-C₁₈alkyl or C₁₄-C₁₈alkenyl; and R₉₃ is -C₂H₄-O(C=O)-C₁₄-C₁₈alkyl or -C₁₄-C₁₈alkenyl, or -C₂H₄-NH(C=O)-C₁₄-C₁₈alkyl or -C₁₄-C₁₈alkenyl.

Other preferred imidazoline cationic fabric softening agents are those having the formula: in which R₉₂ and An^{⊖} have their previous significance; R₉₄ and R₉₅, independently, are a C₈-C₃₀aliphatic residue, C₁-C₄alkyl, C₁-C₄halogenoalkyl, C₁-C₄hydroxyalkyl or a group -C₂H₄-N(R₉₆-C(=O)R₉₇ in which R₉₆ is hydrogen or C₈-C₃₀alkyl and R₉₇ is hydrogen or C₁-C₄alkyl.

Preferably R₉₂ is C₁₄-C₁₈alkyl or C₁₄-C₁₈alkenyl; R₉₄ is C₁₄-C₁₈alkyl, C₁₄-C₁₈alkenyl, C₁-C₄alkyl, C₁-C₄halogenoalkyl or C₁-C₄hydroxyalkyl; and R₉₅ is a group -C₂H₄-N(R₉₆)-C(=O)-R₉₇ in which R₉₆ and R₉₇ have their previous significance.

Preferred anions An^{⊖} include chloride, bromide, iodide, fluoride, sulfate, methosulfate, nitrite, nitrate or phosphate anions, as well as carboxylate anions such as acetate, adipate, phthalate, benzoate, stearate or oleate anions.

Specific examples of preferred compounds of formula (74) include:
2-tallow-1-(2-stearoyloxyethyl)-imidazoline chloride,
2-tallow-1-(2-stearoyloxyethyl)-imidazoline sulfate,
2-tallow-1-(2-stearoyloxyethyl)-imidazoline methosulfate,
2-tallow-1-methyl-3-(2-stearoylamidoethyl)-imidazoline chloride,
2-talow-1-methyl-3-(2-stearoylamidoethyl)-imidazoline sulfate and
2-tallow-1 -methyl-3-(2-stearoylamidoethyl)-imidazoline methosulfate.

Specific examples of preferred compounds of formula (75) include:
2-heptadecyl-1-methyl-1-oleylamidoethyl-imidazolinium-metho-sulfate,
2-heptadecyl-1-methyl-1-(2-stearoylamido)ethyl-imidazolinium-sulfate,
2-heptadecyl-1-methyl-1-(2-stearoylamido)ethyl-imidazolinium- chloride
2-coco-1-(2-hydroxyethyl)-1-benzyl-imidazolinium-chloride
2-coco-1-(2-hydroxyethyl)-1-(4-chlorobutyl)-imidazolinium-chloride
2-coco-1-(2-hydroxyethyl)-1-octadecenyl-imidazolinium-chloride
2-tallow-1-(2-hydroxyethyl)-1-benzyl-imidazolinium-chloride
2-tallow-1-(2-hydroxyethyl)-1-(4-chlorobutyl)-imidazolinium-chloride
2-heptadecenyl-1-(2-hydroxyethyl)-1-(4-chlorobutyl)-imidazolinium-chloride
2-heptadecenyl-1-(2-hydroxyethyl)-1-benzyl-imidazolinium-chloride and
2-heptadecenyl-1-(2-hydroxyethyl)-1-octadecyl-imidazolinium-chloride

One class of preferred quaternary ammonium compounds is that having the formula: in which R₉₈ is a C₈-C₃₀aliphatic residue, R₉₉, R₁₀₀, R₁₀₁, R₁₀₂ and R₁₀₃, independently, are hydrogen, C₁-C₄alkyl or C₁-C₄hydroxyalkyl, An^{⊖} has its previous significance, m₁ is an integer from 1 to 5 and n₂ has its previous significance.

Preferred compounds of formula (76) are those in which R₉₈ is C₁₂-C₁₈alkyl and R₉₉, R₁₀₀, R₁₀₁, R₁₀₂ and R₁₀₃, independently, are C₁-C₄alkyl, especially methyl.

Specific examples of preferred compounds of formula (76) are:
N-(tallow)-N,N,N',N'-tetramethyl-1,3-propanediammoniumdimethosulfate
N-(tallow)-N,N',N'-trimethyl-1,3-propanediammoniumdimetho sulfate
N-(tallow)-N,N',N',N',N'-pentamethyl-1,3-propanediammoniumdimethosulfate
N-oleyl-N,N,N',N',N'-pentamethyl-1,3-propanediammoniumdime thosulfate
N-stearyl-N,N,N',N',N'-pentamethyl-1,3-propanediammoniumdime thosulfate and
N-stearyloxypropyl-N,N',N'-tris(3-hydroxypropyl)-1,3-propanediammoniumdiacetate.

A further class of preferred quaternary ammonium compounds is that having the formula: in which An^{⊖} has its previous significance and the groups R₁₀₄ may be the same or different and each is a C₁-C₃₀aliphatic residue, C₁-C₄hydroxyalkyl, C₂H₄OC(=O)-R₉₂, C₂H₄NHC(=O)-R₉₂ or CH₂CH[OC(=O)-R₉₂][CH₂OC(=O)-R₉₂], in which R₉₂ has its previous significance, provided that at least one group R₁₀₄, and preferably two groups R₁₀₄ are C₁₄-C₃₀alkyl, C₂H₄OC(=O)-C₁₄-C₃₀alkyl, C₂H₄NHC(-O)-C₁₄-C₃₀alkyl or CH₂CH[OC(=O)-C₁₄-C₃₀alkyl][CH₂OC(=O)-C₁₄-C₃₀alkyl]. Preferably, the remaining groups R₁₀₄ are C₁-C₄alkyl, especially methyl or ethyl, or C₁-C₄hydroxyalkyl, especially hydroxymethyl or hydroxyethyl.

Specific examples of preferred compounds of formula (77) are:
distearyldimethylammonium chloride
dilauryldimethylammonium chloride
dihexadecyldimethylammonium chloride
distearyldimethylammonium bromide
distearyldimethylammonium methosulfate and
distearyldi-(isopropyl)-ammonium chloride
distearoyl(hydroxyethyl)methylammonium methosulfate.

Preferred ester amide amine cationic fabric softening agents are those having the formula: in which R₁₀₄ has its previous significance and An₁^{⊖} is an inorganic or organic acid from which an anion An^{⊖} is derived, wherein An^{⊖} has its previous significance, provided that at least one group R₁₀₄, and preferably two groups R₁₀₄ are C₁₄-C₃₀alkyl, (CH₂)ₙOC(=O)-C₁₄-C₃₀alkyl, (CH₂)ₙ₂NHC(=O)-C₁₄-C₃₀alkyl or CH₂CH[OC(=O)-C₁₄-C₃₀alkyl][CH₂OC-C₁₄-C₃₀ alkyl, which n₂ has its previous significance. Preferably, the remaining groups R₁₀₄ are C₁-C₄alkyl, especially methyl or ethyl, or C₁-C₄hydroxyalkyl, especially hydroxymethyl or hydroxyethyl.

A preferred compound of formula (78) is:
3-stearoylamidopropyl-2-stearoyloxymethyl-methylamine hydrochloride.

In addition to the fluorescent whitening agent, the fabric care composition according to the present invention may also contain a minor proportion of one or more adjuvants. Examples of adjuvants include emulsifiers, perfumes, colouring dyes, opacifiers, UV absorbers, bactericides, nonionic surfactants, anti-gelling agents such as nitrites or nitrates of alkali metals, especially sodium nitrate, and corrosion inhibitors such as sodium silicate.

The amount of each of these optional adjuvants should not exceed 2% by weight of the composition.

The present invention also provides, as a yet further aspect, a method for the treatment of a textile article, comprising applying, to a previously washed article, a fabric rinse composition comprising 0.3 to 10% by weight of a cationic, amphoteric or anionic fluorescent whitening agent, based on the total weight of the composition, and optionally a fabric care ingredient, the remainder being substantially water.

Preferably, the fabric care ingredient is a fabric softener, a stain release or stain repellant ingredient or a water-proofing agent, which is preferably present in an amount of from 5 to 25%, especially from 10 to 20% by weight, based on the total weight of the composition.

A preferred method for the treatment of a textile article, comprises applying, to the previously washed article, a rinse cycle fabric softener composition comprising 5 to 25, preferably 10 to 20% by weight of a cationic fabric softening agent and 0.3 to 10, preferably 0.3 to 3% by weight of a cationic, amphoteric or anionic fluorescent whitening agent, each based on the total weight of the composition, the remainder being substantially water.

The use according the present invention, in addition to providing an improvement in the SPF of the treated textile material, may also increase the useful life of the textile material so treated, for example by preserving its tear strength and/or its lightfastness.

The present invention is further illustrated by the following Examples.

### A) Application of a fluorescent whitening agent from a textile treatment composition.

### Examples 1 to 10

An aqueous textile finishing bath is made up having the composition:
2 g/l acetic acid (40%);
40 g/l of an alkyl-modified dihydroxyethyleneurea/melamine-formaldehyde derivative;
12 g/l MgCl₂; and
30 g/l of an emulsion of fatty acid amides.

To separate samples of this bath are added, in the amounts shown in the following Table one or more of the following active substances (AS):

Separate samples of bleached, mercerised cotton (poplin) of density 0.68 g/cm³ and thickness 0.20 mm, are then foularded (70 % liquor uptake) with the various finishing baths, at pH 4-5. Drying of the samples of cotton is effected for 3 minutes at 110°C. followed by thermofixing for 4 minutes at 150°C.

The whiteness (GW) of the treated samples is measured with a DCI/SF 500 spectrophotometer according to the Ganz method. The Ganz method is described in detail in the Ciba-Geigy Review, 1973/1, and also in the article "Whiteness Measurement", ISCC Conference on Fluorescence and the Colorimetry of Fluorescent Materials, Williamsburg, February 1972, published in the Journal of Color and Appearance, 1, No.5 (1972).

The Sun Protection Factor (SPF) is determined by measurement of the UV light transmitted through the swatch, using a double grating spectrophotometer fitted with an Ulbricht bowl. Calculation of SPF is conducted as described by B.L.Diffey and J.Robson in J. Soc. Cosm. Chem. 40 (1989), pp. 130-131.

The results are shown in the following Table 1.

**Table 1**

| Example | AS | Concentration of AS | | GW | SPF |
|---|---|---|---|---|---|
| | | g/l in bath | % on substrate | | |
| - | - | - | - | 62 | 1.9 |
| - | UVA | 10 | 0.35 | 57 | 11.2 |
| - | UVA | 20 | 0.70 | 53 | 17.3 |
| - | UVA | 30 | 1.05 | 34 | 17.4 |
| 1 | UVA | 10 | 0.35 | 175 | 15.8 |
| | FWA-1 | 10 | 0.13 | | |
| 2 | UVA | 20 | 0.70 | 171 | 16.5 |
| | FWA-1 | 10 | 0.13 | | |
| 3 | UVA | 10 | 0.35 | 177 | 18.0 |
| | FWA-1 | 20 | 0.25 | | |
| 4 | UVA | 10 | 0.35 | 167 | 18.3 |
| | FWA-2 | 8 | 0.14 | | |
| 5 | UVA | 20 | 0.70 | 134 | 21.7 |
| | FWA-2 | 8 | 0.14 | | |
| 6 | UVA | 10 | 0.35 | 178 | 15.9 |
| | FWA-2 | 16 | 0.28 | | |
| 7 | FWA-1 | 10 | 0.13 | 227 | 11.7 |
| 8 | FWA-1 | 20 | 0.25 | 229 | 15.2 |
| 9 | FWA-2 | 8 | 0.14 | 223 | 13.0 |
| 10 | FWA-2 | 16 | 0.28 | 215 | 13.2 |

The results in the Table 1 demonstrate clearly the improvement in the SPF value of a substrate treated according to the method of the present invention.

### Examples 11 to 20

Using the general procedure described in Examples 1 to 10, samples of poplin ("Supraluxe" ex Walser AG; density 0.62 g/cm³; thickness 0.17 mm) are foularded (70 % liquor uptake) with the various finishing baths, at pH 4-5. Drying of the samples of poplin is effected for 3 minutes at 110°C. followed by thermofixing for 4 minutes at 150°C.

The whiteness (GW) and SPF of the respective treated samples are measured as before.

In order to evaluate the wash permanency of the textile treatment applied, the respective treated poplin samples are washed ten times and the whiteness (GW) and SPF values are determined after the first, fifth and tenth washes.

50g of the poplin swatches are washed in 1 litre of tap water (12° German hardness) containing 4g of a detergent having the following composition (weight %):

| | |
|---|---|
| 8.0% | Sodium alkylbenzene sulfonate |
| 2.9% | Tallow alcohol-tetradecane-ethylene glycol ether (14 mols EO) |
| 3.5% | Sodium soap |
| 43.8% | Sodium tripolyphosphate |
| 7.5% | Sodium silicate |
| 1.9% | Magnesium silicate |
| 1.2% | Carboxymethyl cellulose |
| 0.2% | EDTA |
| 21.2% | Sodium sulfate |
| x% | fluorescent whitening agent (FWA) by weight on detergent Water to 100%. |

The washing is conducted at 60°C. over 15 minutes. The swatches are then rinsed under cold running tap water for 30 seconds and dried.

The results are set out in the following Table 2.

| Ex. | AS | Concentration of AS | | GW after washing | | | | SPF after washing | | | |
|---|---|---|---|---|---|---|---|---|---|---|---|
| | | g/l in bath | % on sub. | 0x | 1x | 5x | 10x | 0x | 1x | 5x | 10x |
| - | - | - | - | 63 | 71 | 75 | 76 | 4 | 5 | 5 | 5 |
| - | UVA | 10 | 0.35 | 59 | 70 | 69 | 72 | 25 | 18 | 13 | 11 |
| - | UVA | 20 | 0.70 | 55 | 67 | 68 | 71 | 47 | 31 | 30 | 19 |
| - | UVA | 30 | 1.05 | 58 | 68 | 72 | 72 | 81 | 45 | 47 | 30 |
| - | UVA | 40 | 1.40 | 52 | 65 | 70 | 70 | 99 | 46 | 50 | 37 |
| 11 | UVA FWA-1 | 10 10 | 0.35 0.13 | 176 | 152 | 133 | 133 | 57 | 19 | 13 | 10 |
| 12 | UVA FWA-1 | 20 10 | 0.70 0.13 | 147 | 123 | 109 | 108 | 67 | 39 | 24 | 16 |
| 13 | UVA FWA-1 | 10 20 | 0.35 0.25 | 203 | 193 | 160 | 155 | 51 | 19 | 13 | 13 |
| 14 | UVA FWA-2 | 10 8 | 0.35 0.14 | 178 | 178 | 171 | 166 | 41 | 2 | 17 | 19 |
| 15 | UVA FWA-2 | 20 8 | 0.70 0.14 | 149 | 141 | 138 | 136 | 82 | 62 | 34 | 29 |
| 16 | UVA FWA-2 | 10 16 | 0.35 0.28 | 198 | 210 | 208 | 208 | 59 | 26 | 16 | 18 |
| 17 | FWA-1 | 10 | 0.13 | 222 | 205 | 197 | 178 | 24 | 9 | 8 | 7 |
| 18 | FWA-1 | 20 | 0.25 | 236 | 227 | 203 | 209 | 31 | 13 | 6 | 7 |
| 19 | FWA-2 | 8 | 0.14 | 216 | 215 | 216 | 206 | 31 | 19 | 16 | 10 |
| 20 | FWA-2 | 16 | 0.28 | 226 | 239 | 233 | 235 | 42 | 19 | 13 | 16 |

The results in Table 2 demonstrate clearly the improvement in the SPF value of a substrate treated according to the method of the present invention and, moreover, that the use of a combination of UVA and FWA leads to unexpected synergistic SPF values.

### Example 21

A 5 g. sample of poplin ("Supraluxe" ex Walser AG; density 0.62 g/cm³) is foularded (80% liquor uptake) with an aqueous bath containing:
4 g/l sodium bicarbonate and
12.5 g/l of a fluorescent whitening agent having the formula:
to provide a concentration of 1% by weight of active substance on the poplin substrate.

Foularding is conducted at alkaline pH.

Drying of the treated sample is carried out at 80°C. for 2 minutes.

The treated poplin has an SPF rating of above 40, whereas that of the untreated poplin is 4.

### Example 22

A 5 g. sample of poplin ("Supraluxe" ex Walser AG; density 0.62 g/cm³) is foularded (80% liquor uptake) with an aqueous bath containing:
2 g/l acetic acid (40%)
40 g/l of an alkyl-modified dihydroxyethyleneurea/melamine-formaldehyde derivative;
12 g/l MgCl₂;
30 g/l of an emulsion of fatty acid amides and
12.5 g/l of a fluorescent whitening agent having the formula: to provide a concentration of 1% by weight of active substance on the poplin substrate.

Foularding is conducted at a pH of 6-7.

Drying of the treated sample is carried out at 80°C. for 2 minutes, followed by thermofixing for 4 minutes at 150°C.

The treated poplin has an SPF rating of above 30, whereas that of the untreated poplin is 4.

### Example 23

A 5 g. sample of poplin ("Supraluxe" ex Walser AG; density 0.62 g/cm³) is treated with an aqueous bath containing:
3 g/l anhydrous sodium sulfate
3 g/l caustic soda flake
1.5 g/l nonylphenol ethoxylate (7 mols EO) and
1% by weight of poplin fabric of a fluorescent whitening agent having the formula:
the treatment is conducted at 95°C. over 30 minutes and at a liquor ratio of 40:1, using a laboratory dyeing machine.

The treated poplin is rinsed successively with hot or cold water and dried.

The treated poplin has an SPF rating of above 30, whereas that of the untreated poplin is 4.

### B) Application of a fluorescent whitening agent from a detergent composition.

### Examples 24 to 29

50g of bleached, mercerised cotton swatches are washed in 1 litre of tap water (12° German hardness) containing 4g of a detergent having the following composition (weight %):

| | |
|---|---|
| 8.0% | Sodium alkylbenzene sulfonate |
| 2.9% | Tallow alcohol-tetradecane-ethylene glycol ether (14 mols EO) |
| 3.5% | Sodium soap |
| 43.8% | Sodium tripolyphosphate |
| 7.5% | Sodium silicate |
| 1.9% | Magnesium silicate |
| 1.2% | Carboxymethyl cellulose |
| 0.2% | EDTA |
| 21.2% | Sodium sulfate |
| x% | fluorescent whitening agent (FWA) by weight on detergent |
| | Water to 100%. |

The washing is conducted at 40°C. over 15 minutes. The swatches are then rinsed under cold running tap water for 30 seconds and dried. The wash treatment is repeated three times. After the third wash, the swatches are ironed at 160°C.

The results obtained are set out in the following Table 3.

**Table 3**

| Example | FWA | Concentration FWA | W | SPF |
|---|---|---|---|---|
| - | - | - | 79 | 1.6 |
| 24 | Compound (31) | 0.2% | 211 | 6.1 |
| 25 | Compound (32) | 0.2% | 202 | 3.9 |
| 26 | Compound (36) | 0.2% | 200 | 5.2 |
| 27 | Compound (37) | 0.1% | 207 | 4.2 |
| 28 | Compound (40) | 0.1% | 201 | 3.4 |
| 29 | Compound (45) | 0.1% | 208 | 3.1 |

SPF values are the average of 3 measurements at various points on the swatches. The relative variation of the results lies within a range of from about plus or minus 10%.

Compared with the control experiment (no FWA), the SPF values obtained to the invention are 2-4 times higher, after only 3 washes.

### Example 30

A bleached, mercerised cotton swatch is dyed by the exhaustion method using 0.95% by weight on the fabric of a commercial blue reactive dye. The dyeing is conducted at a liquor ratio of 20: 1, the temperature is raised from 25° to 100°C. over 40 minutes, and then held for 1 hour at 100°C. with the addition of 15g/l of sodium sulphate, before applying a final cold rinse.

The SPF of the dyed goods is then determined by the method described in Examples 24 to 29.

The dyed goods are then washed in the manner described in Examples 24 to 29 using the same detergent composition. The FWA compound used in the detergent is the compound of formula (40), at a level of 0.1 weight % of active substance, based on the weight of the detergent. The SPF value of the washed goods and also of goods washed with the same detergent containing no FWA (for control purposes) is determined after 1, 3, 5 and 10 washes. The results are set out in the following Table 4.

**Table 4**

| Example | number of washes | SPF | |
|---|---|---|---|
| | | without fwa | with fwa |
| - | control pre-wash | 23.7 | 23.7 |
| 30 | one | 22.5 | 23.8 |
| | three | 22.0 | 25.9 |
| | five | 20.9 | 26.9 |
| | ten | 19.8 | 28.7 |

The results in Table 4 demonstrate that the SPF of dyed fabrics can decrease significantly when the fabrics are washed with a detergent which does not contain an FWA. By contrast, washing with a detergent containing a compound of formula (40) not only eliminates this loss of protection against aggressive sunlight radiation, but also actually increases the SPF protection with successive washings.

### C) Application of a fluorescent whitening agent from a rinse composition.

### Example 31

The following rinse cycle softener base composition is made up:
7.0g. distearyldimethylammonium chloride (72% active ingedient)
0.5g. fatty alcohol ethoxylate
92.5g. deionised water.

To this is added 0.3g., 0.9g. or 2.7g., respectively, of the amphoteric fluorescent whitening agent of formula:

### Example 32

The following rinse cycle softener base composition is made up:
7.0g. distearyldimethylammonium chloride
0.5g. fatty alcohol ethoxylate
92.5g. deionised water.

To this is added 0.3g., 0.9g. or 2.7g., respectively, of the cationic fluorescent whitening agent of formula:

### Examples 33 and 34

5g. of cotton fabric are first washed with 4g/l of ECE standard detergent using a liquor ratio of 1:20 at 60°C. The washed goods are then rinsed and are subjected, while still wet, to a rinse softener treatment. The amount of the rinse cycle softener base composition of Example 1 or 2 used is 5g/l. The liquor ratio is 1:40 using tap water and the treatment is effected at 25°C. for 10 minutes. The softener-treated goods are then spin-dried at 60°C.

The whiteness and SPF values of the dried softener-treated goods are measured.

The dried softener-treated goods are then re-washed using the same detergent and washing conditions that are used for the initial wash except that, after the rinse, the re-washed goods are spin-dried at 60°C. without being subjected to a rinse softener treatment. The whiteness and SPF values of the re-washed, dried goods are measured.

The results are shown in the following Table 5.

**Table 5**

| Example | Rinse Composition | Conc. FWA | Without re-wash | | With re-wash | |
|---|---|---|---|---|---|---|
| | | | GW | SPF | GW | SPF |
| - | control (no FWA) | - | 67 | 3 | 75 | 3 |
| 33 | Rinse of Example 31 | 0.3 | 194 | 9 | 181 | 8 |
| | | 0.9 | 197 | 15 | 199 | 11 |
| | | 2.7 | 169 | 24 | 200 | 16 |
| 34 | Rinse of Example 32 | 0.3 | 199 | 14 | 182 | 13 |
| | | 0.9 | 206 | 17 | 202 | 20 |
| | | 2.7 | 193 | 29 | 193 | 26 |

The concentration of FWA denotes the concentration of active FWA compound based on the total weight of the rinse formulation.

The results in Table 5 clearly demonstrate the improvement in the Ganz Whiteness and SPF values of a cotton substrate treated with a rinse composition according to the present invention, both before and after a subsequent re-wash.

Similar results are obtained when the fluorescent whitening agent used in Example 31 or 32 is replaced by a compound having one of the following formulae:

## Claims

1. Use of a fluorescent whitening agent for improving the sun protection factor (SPF) of textile fibre material, wherein said fluorescent whitening agent absorbs radiation in the wavelength range 280-400 nm, in a composition which is
a) an aqueous textile finishing composition;
comprising at least one fluorescent whitening agent which is selected from the group consiting of :4,4'-bis-(triazinylamino)-stilbene-2,2'-disulfonic acid, 4,4'-bis-(triazol-2-yl)stilbene-2,2'-disulfonic acid, 4,4'-(diphenyl)-stilbenes, 4,4'-distyryl-biphenyl, 4-phenyl-4'-benzoxazolyl-stilbene, stilbenyl-naphthotriazoles, 4-styryl-stilbene, bis-(benzoxazol-2-yl) derivatives, bis-(benzimidazol-2-yl) derivative, coumarine, pyrazoline, naphthalimide, triazinyl-pyrene, 2-styryl-benzoxazole- or -naphthoxazole derivative, benzimidazole-benzofuran or oxanilide derivative, or
b) a detergent composition
comprising at least one fluorescent whitening agent, which is selected from the group consiting of: in which R₄₃ and R₄₄, independently, are OH, NH₂, O-C₁-C₄-alkyl, O-aryl, NH-C₁-C₄-alkyl, N(C₁-C₄-alkyl)₂, N(C₁-C₄-alkyl)(C₁-C₄hydroxyalkyl), N(C₁-C₄-hydroxyalkyl)₂, NH-aryl, morpholino, S-C₁-C₄-alkyl(aryl), Cl or OH; R₄₅ and R₄₆, independently, are H, C₁-C₄-alkyl, phenyl or a group of formula: R₄₇ is H, Cl or SO₃M; R₄₈ is CN, SO₃M, S(C₁-C₄-alkyl)₂ or S(aryl)₂; R₄₉ is H, SO₃M, O-C₁-C₄-alkyl, CN, Cl, COO-C₁-C₄-alkyl, or CON(C₁-C₄-alkyl)₂; R₅₀ is H, C₁-C₄-alkyl, Cl or SO₃M; R₅, and R₅₂, independently, are H, C₁-C₄-alkyl, SO₃M, Cl or O-C₁-C₄-alkyl; R₅₃ is H or C₁-C₄-alkyl; R₅₄ is H, C₁-C₄-alkyl, CN, Cl, COO-C₁-C₄-alkyl, CON(C₁-C₄-alkyl)₂, aryl or O-aryl;
and
M is H, Na, K, Ca, Mg, ammonium, mono-, di-, tri- or tetra- C₁-C₄-alkyl ammonium, mono-, di- or tri- C₁-C₄-hydroxyalkylammonium or ammonium that is di- or tri-substituted by a mixture of C₁-C₄-alkyl and C₁-C₄-hydroxyalkyl groups, and n is 0 or 1;
or
c) a post-wash fabric care composition comprising at least a fluorescent whitening agent,
wherein said fluorescent whitening agent is a cationic bistyrylphenyl fluorescent whitening agent of formula: in which Y is arylene, optionally substituted by chloro, methyl or methoxy; q is 1 or 2; R₅₅ is hydrogen, chloro, C₁-C₄-alkyl, C₁-C₄-alkoxy, cyano or C₁-C₄-alkoxycarbonyl; R₅₆ and R₅₇ are C₁C₄-alkyl, chloroethyl, methoxyethyl, beta -ethoxyethyl, beta -acetoxyethyl or beta - cyanoethyl, benzyl or phenylethyl; R₅₈ is C₁-C₄-alkyl, C₂-C₃-hydroxyalkyl, beta -hydroxy- gamma -chloropropyl, beta -cyanoethyl or C₁₋C₄-alkoxy-carbonylethyl; and An(⁻) is an anion of an organic or anionic acid; or,
a cationic bistyrylphenyl fluorescent whitening agent of formula: in which R₅₅ and q have their previous significance and Y₁ is C₂-C₄-alkylene or hydroxypropylene; R₅₉ is C₁-C₄-alkyl or, together with R₆₀ and the nitrogen to which they are each attached, R₅₉ forms a pyrrolidine, piperidine, hexamethyleneimine or morpholine ring; R₆₀ is C1-C4-alkyl or, together with R₅₉ and the nitrogen to which they are each attached, R₆₀ forms a pyrrolidine, piperidine, hexamethyleneimine or morpholine ring; R₆₁ is hydrogen, C₁-C₄-alkyl, C₃-C₄-alkenyl, C₁-C₄-akoxycarbonylmethyl, benzyl, C₂-C₄-hydroxyalkyl, C₂-C₄-cyanoalkyl or, together with R₅₉ and R₆₀ and the nitrogen atom to which they are each attached, R₆₁ forms a pyrrolidine, piperidine, hexamethyleneimine or morpholine ring, and p is 0 or 1 and An(-) is an anioin of an organic or inorganic acid; or,
a bistyrylphenyl fluorescent whitening agent of formula: in which R₅₅, Y₁, p and q have their previous significance and An(-) is an anioin of an organic or inorganic acid, and R₆₂ and R₆₃, independently, are C₁-C₄-alkyl or C₂-C₃-alkenyl or R₆₂ and R₆₃, together with the nitrogen atom to which they are attached, form a pyrrolidine, piperidine, hexamethyleneimine or morpholine ring; R₆₄ is hydrogen, C₁-C₄-alkyl or C₂-C₃-alkenyl or R₆₂. R₈₃ and R₆₄, together with the nitrogen atom to which they are attached, form a pyridine or picoline ring; and Z is sulfur, -SO₂-, -SO₂NH-, -O-C₁-C₄-alkylene-COO- or -OCO-, or, in which the cationic bistyrylphenyl fluorescent whitening agent has the formula: in which R₅₅, R₆₂, R₆₃, R₆₄, Y₁, p and q have their previous significance and An(-) is an anioin of an organic or inorganic acid; or, a amphoteric styrene fluorescent whitening agent offormula: in which R₅₅, R₆₂, R₆₃, Y₁, and q have their previous significance and An(-) is an anioin of an organic or inorganic acid; Z₁ is oxygen, sulfur, a direct bond, -COO-, -CON(R₆₅)- or -SO₂N(R₆₅)- in which R₆₅ is hydrogen, C₁-C₄-alkyl or cyanoethyl; and Q is -COO-or -SO₃, and, in which the amine oxide fluorescent whitening agent has the formula: in which in which q has its previous significance and B is a brightener radical selected from a 4,4'-distyrylbiphenyl, 4,4'-divinyl-stilbene, and a 1,4'-distyrylbenzene, each optionally substituted by one to four substituents selected from halogen, C₁-C₄-alkyl, C₁-C₄-hydroxyalkyl, C₁-C₄-halogenoalkyl, C₁-C₄-cyanoalkyl, C₁-C₄-alkoxy- C₁-C₄-alkyl, phenyl- C₁-C₄-alkyl, carboxy- C₁-C₄-alkyl, carb- C₁-C₄-alkoxy- C₁-C₄-alkyl, C₁-C₄-alkenyl, C₅-C₈-cycloalkyl, C₁-C₄-alkoxy, C₁-C₄-alkenoxy, C₁-C₄-alkoxycarbonyl, carbamoyl, cyano, C₁-C₄-alkyl-sulfonyl, phenylsulfonyl, C₁-C₄-alkoxysulfonyl, sulfamoyl, hydroxyl, carboxyl, sulfo and trifluoromethyl;Z₂ is a direct bond between B and Y₂, an oxygen atom, a sulfur atom, -SO₂-, -SO₂-O-, -COO-, -CON(R₆₈)- or -SO₂N(R₆₈)- in which R₆₈ is hydrogen or C₁-C₄-alkyl optionally substituted by halogen, cyano, hydroxyl, C₂-C₅-carbalkoxy, C₁-C₄-alkoxy, phenyl, chlorophenyl, methylphenyl, methoxyphenyl, carbamoyl or sulfamoyl; Y₂ is C₂-C₄-alkylene or C₂-C₄-alkyleneoxy-C₂-C₄-alkylene, each optionally substituted by halogen, hydroxyl, C₂-C₅-carbalkoxy, C₁-C₄-alkoxy, phenyl, chlorophenyl, methylphenyl, methoxyphenyl, carbamoyl or sulfamoyl; and R₆₆ and R₆₇, independently, are C₅-C₈-cycloalkyl, C₁-C₄-alkyl or phenyl, each optionally substituted by halogen, hydroxyl, C₂-C₅-carbalkoxy, C₁-C₄-alkoxy, phenyl, chlorophenyl, methylphenyl, methoxyphenyl, carbamoyl or sulfamoyl; in which, in all the carbamoyl or sulfamoyl groups, the nitrogen atom is optionally substituted by one or two C₁-C₄-alkyl, C₁-C₄-hydroxyalkyl, C₂-C₅-cyanoalkyl, C₁-C₄-halogenoalkyl, benzyl or phenyl groups, or,
a cationic fluorescent whitening agent of formula: in which Y₂ and q have their previous significance and B₁ is brightener radical; Z₃ is a direct bond, -SO₂-C₂-C₄₋alkyleneoxy, -SO₂-C₂-C₄-alkylene-COO-, -SO₂, -COO-, -SO₂-C₂-C₄-alkylene-CON(R₇₅)- or -SO₂N(R₇₅)- in which R₇₅ is hydrogen or C₁-C₄-alkyl optionally substituted by hydroxyl, halogen or cyano; R₇₀ is C₁-C₄-alkyl or C₂-C₄-alkenyl, each optionally substituted by halogen, cyano, hydroxy, C₁-C₄-alkoxycarbonyl or C₁-C₄-alkylcarbonyloxy, or R₇₀ is benzyl, optionally substituted by halogen, C₁-C₄-alkyl or C₁-C₄-alkoxy, or R₇₀, together with R₇₁ or Z₃, forms a pyrrolidine, piperidine or morpholine radical;R₇₁ is C₁-C₄-alkyl or C2-C4-alkenyl, each optionally substituted by halogen, cyano, hydroxy, C₁-C₄-alkoxycarbonyl or C₁-C₄-alkylcarbonyloxy, or R₇₁ is benzyl, optionally substituted by halogen, C₁-C₄-alkyl or C₁-C₄-alkoxy, or R₇₁, together with R₇₀, forms a pyrrolidine, piperidine or morpholine radical; R₇₂ is C₁-C₄-alkyl; R₇₃ is hydrogen or
C₁-C₄-alkyl, optionally substituted by cyano, hydroxy, C₁-C₄-alkoxycarbonyl or C₁-C₄-alkylcarbonyloxy; and R₇₄ is C₁-C₄-alkyl, or,
wherein said fluorescent whitening agent is a bis(triazinyl)diaminostilbene anionic fluorescent whitening agent of formula: or a dibenzofuranylbiphenyl anionic fluorescent whitening agent of formula: and or an anionic bistyrylphenyl fluorescent of formula: in which R₇₆ is phenyl optionally substituted by one or two SO₃M groups and R₇₇ is NH- C₁-C₄-alkyl, N(C₁-C₄-alkyl)₂, NH- C₁-C₄-alkoxy, N(C₁-C₄-alkoxy)₂, N(C₁-C₄-alkyl)( C₁-C₄-hydroxyalkyl), N(C₁-C₄-hydroxyalkyl)₂; R₇₀ is H, C₁-C₄-alkyl, CN, Cl or SO₃M; R₇₉ and R₈₀, independently, are H, C₁-C₄-alkyl, SO₃M, CN, Cl or O- C₁-C₄-alkyl, provided that at least two of R₇₈, R₇₉ and R₈₀ are SO3M and the third group has solubilising character; R₈₁ is H, SO₃M, O- C₁-C₄-alkyl, CN, Cl, COO- C₁-C₄-alkyl, or CON(C₁-C₄-alkyl)₂; and r is 0 or 1 and M has its previous significance.

2. Use according to claim 1, in which the composition is an aqueous textile finishing composition and the amount of fluorescent whitening agent present in the composition ranges from 0.01 to 3%; or the composition is a detergent composition and the amount of fluorescent whitening agent present in the composition ranges from 0.005 to 2%.

3. Use according to claim 1, in which the composition is an aqueous textile finishing composition and the fluorescent whitening agent used is a the 4,4'-bis-(triazinylamino)-stilbene-2,2'-disulfonic acid is one having the formula: in which R₁ and R₂, independently, are phenyl, mono- or disulfonated phenyl, phenylamino, mono- or disulfonated phenylamino, morpholino, -N(CH₂CH₂OH)₂, -N(CH₃)(CH₂CH₂OH), -NH₂, -N(C₁-C₄-alkyl)₂, -OCH₃, -Cl, -NH-CH₂CH₂SO₃H or -NH-CH₂CH₂OH; and M is H, Na, K, Ca, Mg, ammonium, mono-, di-, tri- or tetra-C₁-C₄-alkylammonium, mono-, di- or tri-C₁-C₄-hydroxyalkylammonium or ammonium that is di- or tri-subsiituted with by a mixture of C₁-C₄-alkyl and C₁-C₄-hydroxyalkyl groups, and,
in which the 4,4'-bis-(triazol-2-yl)stilbene-2,2'-disulfonic acid is one having the formula: in which R₃ and R₄, independently, are H, C₁-C₄-alkylphenyl or monosulfonated phenyl, and, in which the 4,4'-(diphenyl)-stilbene is one having the formula: and,
in which the 4,4'-distyryl-biphenyl used has the formula: in which R₅ and R₆, independently, are H, SO₃M, SO₂N(C₁-C₄-alkyl)₂, O-(C₁-C₄-alkyl), CN, Cl, COO(C₁-C₄-alkyl), CON(C₁-C₄-alkyl)₂ or O(CH₂)₃N(+)(CH₃)₂An(-), in which An(-) is an anion of an organic or inorganic acid; and n is 0 or 1, or in which the 4-phenyl-4'-benzoxazolylstilbene has the formula: in which R₇ and R₈, independently, are H, Cl, C₁-C₄-alkyl or SO₂-C₁-C₄-alkyl, and,
in which a stilbenyl-naphthotriazole used is one of formula in which R₉ is H or Cl; R₁₀ is SO₃M, SO₂N(C₁-C₄-alkyl)₂, SO₂O-phenyl or CN; R₁₁ is H or SO₃M, and in which a 4-styryl-stilbene used is one of formula: in which R₁₂ and R₁₃, independently, are H, SO₃M, SO₂N(C₁-C₄-alkyl)₂, O-(C₁-C₄-alkyl), CN, Cl, COO(C₁-C₄-alkyl), CON(C₁-C₄-alkyl)₂ or O(CH₂)₃N(+)(CH₃)₂An(-), and
in which a bis-(benzoxazol-2-yl) derivative used having the formula: in which R₁₄, independently, is H, C(CH₃)₃, C(CH₃)₂-phenyl, C₁-C₄-alkyl or COO-C₁-C₄-alkyl, and X is -CH=CH- or a group of formula: and in which a bis-(benzimidazol-2-yl) derivatives is used of formula: in which R₁₅ and H₁₆, independently, are H, C₁-C₄-alkylor CH₂CH₂OH, R₁₇ is H or SO₃M; X₁ is - CH =CH- or a group of formula: and in which a coumarine is used of formula: in which R₁₈ is H, Cl or CH₂COOH, R₁₉ is H, phenyl, COO-C₁-C₄-alkyl or a group of formula: and R₂₀ is O-C₁-C₄-alkyl, N(C₁-C₄-alkyl)₂, NH-CO-C₁-C₄-alkyl or a group of formula: or in which R₂₁ is H, C₁-C₄-alkyl or phenyl, and,
in which a pyrazoline used is one having the formula: in which R₂₂ is H, Cl or N(C₁-C₄-alkyl)₂, R₂₃ is H, Cl, SO₃M, SO₂NH₂, SO₂NH-(C₁-C₄-alkyl), COO-C₁-C₄-alkyl, SO₂C₁-C₄-alkyl, SO₂NHCH₂CH₂CH₂N(⁺)(CH₃)₃ or SO₂CH₂CH₂N(⁺)H(C₁-C₄-alkyl)₂ An(⁻), R₂₄ and R₂₅ are the same or different and each is H, C₁-C₄-alkyl or phenyl and R₂₆ is H or Cl; and
in which a naphthalimide is used of formula: in which R₂₇ is C₁-C₄-alkyl or CH₂CH₂CH₂N(⁺)(CH₃)₃; R₂₈ is O- C₁-C₄-alkyl, SO₃M or NH-CO-C₁-C₄-alkyl;and,
in which a triazinyl-pyrene is used of formula: in which each R₂₉, independently, is C₁-C₄-alkoxy, and
in which a 2-styryl-benzoxazole- or -naphthoxazole derivative is used having the formula: in which R₃₁ is CN, Cl, COO-C₁-C₄-alkyl or phenyl; R₃₂ and R₃₃ are the atoms required to form a fused benzene ring or R₃₃ and R₃₅, independently, are H or C₁-C₄-alkyl; and R₃₄ is H, C₁-C₄-alkyl or phenyl, and,
in which a benzimidazole-benzofuran derivative is used having the formula: in which R₃₆ is C₁-C₄-alkoxy; R₃₇ and R₃₈, independently, are C₁-C₄-alkyl
and in which an oxanilide derivative is used having the formula: in which R₃₉is C₁-C₄alkoxy, R₄₁ is C₁-C₄alkyl, C₁-C₄alkyl-SO₃M or C₁-C₄alkoxy -SO₃M iand R₄₀ and R₄₂ are the same and each is hydrogen, tert. butyl or SO₃M.

4. Use according to any of claim 1, in which the composition is a textile finishing composition and the fluorescent whitening agent is used:
a) in mixtures with dyes (shading) or pigments;
b) in mixtures with carriers, wetting agents, antioxidants, UV absorbers and/or chemical bleaching agents; or
c) in admixture with crosslinking or finishing agents or in combination with a textile finishing process or flameproof finish, soft handle finish, antisoiling finish, antistatic finish or antimicrobial finish.

5. Use according to claim 1, in which the compound of formula (23) has the formula: or
in which the compound of formula (24) has the formula: in which n is as defined in claim 1;
in which the compound of formula (26) has the formula: or
in which the compound of formula (27) has the formula: or
in which the compound of formula (30) has the formula:

6. Use according to claim 1, in which the compound of formula (56) has the formula (31), (32) or (34), or in which the compound of formula (57) has the formula (43), (44), (45) or (46), or in which the compound of formula (58) has the formula (40), (41) or (42), each as defined in claim 5.

7. Use according to claim 1, wherein the used composition is a detergent composition comprising:
i) 5-90% of an anionic surfactant and/or a nonionic surfactant;
ii) 5-70% of a builder;
iii) 0-30% of a peroxide;
iv) 0-10% of a peroxide activator and/or 0-1% of a bleaching catalyst;
v) 0.005-2% of at least one fluorescent whitening agent which absorbs radiation in the wavelength range 280-400 nm; and
vi) 0.005-10% of one or more auxiliaries, each by weight, based on the total weight of the detergent.

8. A stable, concentrated rinse cycle fabric softener composition comprising 2 to 25 % by weight of a fabric softener agent, and >0.3 to 10 % by weight of a fluorescent whitening agent which is compatible with the fabric softener agent, each based on the total weight of the composition, the remainder being substantially water.

9. Process for the treatment of a textile article, comprising applying, to a previously washed article, a fabric rinse composition comprising >0.3 to 10% by weight of a cationic, amphoteric or anionic fluorescent whitening agent, based on the total weight of the composition, and optionally a fabric care ingredient, the remainder being substantially water.

## Patentansprüche

1. Verwendung eines fluoreszierenden Weißmachers zur Verbesserung des Sonnenschutzfaktors (SPF) von Textilfasermaterialien, worin der fluoreszierende Weißmacher die Strahlung in dem Wellenlängenbereich von 280 - 400 nm absorbiert, in einer Zusammensetzung, welche darstellt
a) eine wässrige Textilappreturzusammensetzung;
umfassend mindestens einen fluoreszierenden Weißmacher, welcher ausgewählt ist aus der Gruppe, bestehend aus: 4,4'-Bis-(triazinylamino)-stilben-2,2'-disulfonsäure, 4,4'-Bis-(triazol-2-yl)stilben-2.2'-disulfonsäure, 4.4'-(Diphenyl)-stilbenen. 4,4'-Distyryl-biphenyl, 4-Phenyl-4'-benzoxazolyl-stilben, Stilbenyl-naphthotriazolen, 4-Styryl-stilben, Bis-(benzoxazol-2-yl)-Derivaten, Bis-(benzimidazol-2-yl)-Derivaten, Coumarin, Pyrazolin, Naphthalimid, Triazinyl-pyren, 2-Styryl-benzoxazoloder -naphthoxazol-Derivaten, Benzimidazol-benzofuran- oder Oxanilid-Derivaten, oder
b) eine Reinigungmittelszusammensetzung,
umfassend mindestens einen fluoreszierenden Weißmacher, welcher ausgewählt ist aus der Gruppe, bestehend aus: worin R₄₃ und R₄₄ unabhängig voneinander OH, NH₂, O-C₁-C₄-Alkyl, O-Aryl, NH-C₁-C₄-Alkyl, N(C₁-C₄-Alkyl)₂, N(C₁-C₄-Alkyl)((C₁-C₄-hydroxyalkyl). N(C₁-C₄-Hydroxyalkyl)₂, NH-Aryl, Morpholino, S-C₁-C₄-Alkyl(aryl). Cl oder OH darstellen; R₄₅ und R₄₆ unabhängig voneinander H, C₁-C₄-Alkyl, Phenyl oder eine Gruppe der Formel: darstellen; R₄₇ H, Cl oder SO₃M ist; R₄₈ CN, SO₃M, S(C₁-C₄-Alkyl)₂ oder S(Aryl)₂ ist; R₄₉ H, SO₃M, O-C₁-C₄-Alkyl, CN, Cl, COO-C₁-C₄-Alkyl oder CON(C₁-C₄-Alkyl)₂ darstellt; R₅₀ H, C₁-C₄-Alkyl, Cl oder SO₃M ist; R₅₁ und R₅₂ unabhängig voneinander H, C₁-C₄-Alkyl, SO₃M, Cl oder O-C₁-C₄-Alkyl sind; R₅₃ H oder C₁-C₄-Alkyl ist; R₅₄ H, C₁-C₄-Alkyl, CN, Cl, COO-C₁-C₄-Alkyl, CON(C₁-C₄-Alkyl)₂, Aryl oder 0-Aryl darstellt;
und
M H, Na, K, Ca, Mg, Ammonium, Mono-, Di-, Tri- oder Tetra-C₁-C₄-alkylammonium, Mono-, Di- oder Tri-C₁-C₄-hydroxyalkylammonium oder Ammonium darstellt, welches di- oder trisubstituiert ist durch eine Mischung von C₁-C₄-Alkyl- und C₁-C₄-Hydroxyalkylgruppen, und n 0 oder 1 ist;
oder
c) eine post-Wasch-Textilpflegezusammensetzung, umfassend mindestens einen fluoreszierenden Weißmacher,
worin der fluoreszierende Weißmacher einen kationischen fluoreszierenden Bistyrylphenyl-Weißmacher der Formel darstellt: worin Y Arylen, wahlweise substituiert durch Chlor, Methyl oder Methoxy, darstellt; q 1 oder 2 ist; R₅₅ Wasserstoff, Chlor, C₁-C₄-Alkyl, C₁-C₄-Alkoxy. Cyano oder C₁-C₄-Alkoxycarbonyl ist; R₅₆ und R₅₇ C₁-C₄-Alkyl, Chlorethyl, Methoxyethyl, beta-Ethoxyethyl, beta-Acetoxyethyl oder beta-Cyanoethyl, Benzyl oder Phenylethyl darstellen; R₅₈ C₁-C₄-Alkyl, C₂-C₃-Hydroxyalkyl. beta-Hydroxy-gammachlorpropyl, beta-Cyanoethyl oder C₁-C₄-Alkoxycarbonylethyl ist; und An(⁻) ein Anion einer organischen oder anorganischen Säure darstellt; oder
ein kationischer fluoreszierender Bistyrylphenyl-Weißmacher der Formel ist: worin R₅₅ und q deren vorstehende Bedeutung aufweisen und Y₁ C₂-C₄-Alkylen oder Hydroxypropylen ist: R₅₉ C₁-C₄-Alkyl ist oder R₅₉ zusammen mit R₆₀ und dem Stickstoff, an den sie jeweils gebunden sind, einen Pyrrolidin-, Piperidin-, Hexamethylenimin- oder Morpholinring bildet; R₆₀ C₁-C₄-Alkyl darstellt oder R₆₀ zusammen mit R₅₉ und dem Stickstoff, an den sie jeweils gebunden sind, einen Pyrrolidin-, Piperidin-, Hexamethylenimin- oder Morpholinring bildet; R₆₁ Wasserstoff, C₁-C₄-Alkyl, C₃-C₄-.Alkenyl, C₁-C₄-Alkoxycarbonylmethyl, Benzyl, C₂-C₄-Hydroxyalkyl, C₂-C₄-Cyanoalkyl ist oder R₆₁ zusammen mit R₅₉ und R₆₀ und dem Stickstoffatom, an das sie jeweils gebunden sind, einen Pyrrolidin-, Piperidin-, Hexamethylenimin- oder Morpholinring bildet, und p 0 oder 1 ist und An(⁻) ein Anion einer organischen oder anorganischen Säure darstellt; oder
ein fluoreszierender Bistyrylphenyl-Weißmacher der Formel ist: worin R₅₅, Y₁, p und q deren vorstehende Bedeutung aufweisen und An(-) ein Anion einer organischen oder anorganischen Säure ist und R₆₂ und R₆₃ unabhängig voneinander C₁-C₄-Alkyl oder C₂-C₃-Alkenyl sind oder R₆₂ und R₆₃ zusammen mit dem Stickstoffatom, an welches sie gebunden sind. einen Pyrrolidin-, Piperidin-, Hexamethylenimin- oder Morpholinring bilden; R₆₄ Wasserstoff, C₁-C₄-Alkyl oder C₂-C₃-Alkenyl ist oder R₆₂, R₆₃ und R₆₄ zusammen mit dem Stickstoffatom, an welches sie gebunden sind, einen Pyridin- oder Picolinring bilden; und Z Schwefel, -SO₂-, -SO₂NH-, -O- C₁-C₄-Alkylen-COO- oder -OCO- darstellt, oder worin der kationische fluoreszierende Bistyrylphenyl-Weißmacher die Formel aufweist: worin R₅₅, R₆₂. R₆₃, R₆₄, Y₁, p und q deren vorstehende Bedeutung aufweisen und An(-) ein Anion einer organischen oder anorganischen Säure darstellt; oder
ein amphoterer fluoreszierender Styrol-Weißmacher der Formel ist: worin R₅₅, R₆₂, R₆₃, Y₁ und q deren vorstehende Bedeutung aufweisen und An(-) ein Anion einer organischen oder anorganischen Säure darstellt; Z₁ Sauerstoff. Schwefel, eine direkte Bindung, -COO-, -CON(R₆₅)- oder -SO₂N(R₆₅)- darstellt,
worin R₆₅ Wasserstoff, C₁-C₄-Alkyl oder Cyanoethyl ist; und Q -COO- oder -SO₃ ist, und
worin der fluoreszierende Aminoxid-Weichmacher die Formel aufweist: worin q dessen vorstehende Bedeutung aufweist und B einen Aufhellerrest darstellt, ausgewählt aus 4,4'-Distyrylbiphenyl, 4,4'-Divinylstilben und einen 1,4'-Distyrylbenzol, jeweils wahlweise substituiert durch ein bis vier Substituenten, ausgewählt aus Halogen, C₁-C₄-Alkyl, C₁-C₄-Hydroxyalkyl, C₁-C₄-Halogenalkyl, C₁-C₄-Cyanoalkyl, C₁-C₄-Alkoay-C₁-C₄-alkyl, Phenyl-C₁-C₄-alkyl, Carboxy-C₁-C₄alkyl, Carb-C₁-C₄-alkoxy-C₁-C₄-alkyl, C₁-C₄-Alkenyl, C₅-C₈-Cycloalkyl, C₁-C₄-Alkoxy, C₁-C₄-Alkenoxy, C₁-C₄-Alkoxycarbonyl, Carbamoyl, Cyano, C₁-C₄-Alkylsulfonyl, Phenylsulfonyl, C₁-C₄-Alkoxysulfonyl, Sulfamoyl, Hydroxyl, Carboxyl, Sulfo und Trifluormethyl; Z₂ eine direkte Bindung zwischen B und Y₂, ein Sauerstoffatom, ein Schwefelatom, -SO₂-, -SO₂-O-, -COO-, -CON(R₆₈)- oder -SO₂N(R₆₈)-darstellt, worin R₆₈ Wasserstoff oder C₁-C₄-Alkyl darstellt, wahlweise substituiert durch Halogen, Cyano, Hydroxyl, C₂-C₅-Carbalkoxy, C₁-C₄-Alkoxy, Phenyl, Chlorphenyl, Methylphenyl, Methoxyphenyl, Carbamoyl oder Sulfamoyl; Y₂ C₂-C₄-Alkylen oder C₂-C₄-Alkylenoxy-C₂-C₄-alkylen ist, jeweils wahlweise substituiert durch Halogen, Hydroxyl, C₂-C₅-Carbalkoxy, C₁-C₄-Alkoxy, Phenyl, Chlorphenyl, Methylphenyl, Methoxyphenyl, Carbamoyl oder Sulfamoyl; und R₆₆ und R₆₇ unabhängig voneinander C₅-C₈-Cycloalkyl, C₁-C₄-Alkyl oder Phenyl darstellen, jeweils wahlweise substituiert durch Halogen, Hydroxyl, C₂-C₅-Carbalkoxy, C₁-C₄-Alkoxy, Phenyl, Chlorphenyl. Methylphenyl, Methoxyphenyl, Carbamoyl oder Sulfamoyl;
worin in allen Carbamoyl- oder Sulfamoylgruppen das Stickstoffatom wahlweise substituiert ist durch eine oder zwei C₁-C₄-Alkyl-, C₁-C₄-Hydroxyalkyl-, C₂-C₅-Cyanoalkyl-, C₁-C₄-Halogenalkyl-, Benzyl- oder Phenylgruppen, oder
ein kationischer fluoreszierender Weißmacher der Formel ist: worin Y₂ und q deren vorstehende Bedeutung aufweisen und B₁ ein Aufhellerrest darstellt; Z₃ eine direkte Bindung, -SO₂- C₂-C₄-Alkylenoxy, -SO₂- C₂-C₄-Alkylen-COO-. -SO₂-, -COO-, -SO₂-C₂-C₄-Alkylen-CON(R₇₅)- oder -SO₂N(R₇₅)- ist, worin R₇₅ Wasserstoff oder C₁-C₄-Alkyl darstellt, wahlweise substituiert durch Hydroxyl. Halogen oder Cyano; R₇₀ C₁-C₄-Alkyl oder C₂-C₄-Alkenyl ist, jeweils wahlweise substituiert durch Halogen, Cyano, Hydroxy, C₁-C₄-Alkoxycarbonyl oder C₁-C₄-Alkylcarbonyloxy, oder R₇₀ Benzyl ist, wahlweise substituiert durch Halogen, C₁-C₄-Alkyl oder C₁-C₄-Alkoxy, oder R₇₀ zusammen mit R₇₁ oder Z₃ einen Pyrrolidin-, Piperidin- oder Morpholinrest bildet; R₇₁ C₁-C₄-Alkyl oder C₂-C₄-Alkenyl darstellt, jeweils wahlweise substituiert durch Halogen, Cyano, Hydroxy, C₁-C₄-Alkoxycarbonyl oder C₁-C₄-Alkylcarbonyloxy, oder R₇₁ Benzyl ist, wahlweise substituiert durch Halogen, C₁-C₄-Alkyl oder C₁-C₄-Alkoxy, oder R₇₁ zusammen mit R₇₀ einen Pyrrolidin-, Piperidin- oder Morpholinrest bildet; R₇₂ C₁-C₄-Alkyl ist; R₇₃ Wasserstoff oder C₁-C₄-Alkyl darstellt, wahlweise substituiert durch Cyano, Hydroxy, C₁-C₄-Alkoxycarbonyl oder C₁-C₄-Alkylcarbonyloxy; und R₇₄ C₁-C₄-Alkyl ist, oder
worin der fluoreszierende Weißmacher einen anionischen fluoreszierenden Bis(triazinyl)diaminostilben-Weißmacher der Formel darstellt: oder ein anionischer fluoreszierender Dibenzofuranylbiphenyl-Weißmacher der Formel ist: und oder ein anionischer fluoreszierender Bistyrylphenyl-Weißmacher der Formel ist: worin R₇₆ Phenyl darstellt, wahlweise substituiert durch eine oder mehrere SO₃M-Gruppen, und R₇₇ NH-C₁-C₄-Alkyl, N(C₁-C₄-Alkyl)₂, NH-C₁-C₄-Alkoxy, N(C₁-C₄-Alkoxy)₂, N(C₁-C₄-Alkyl)(C₁-C₄-hydroxyalkyl), N(C₁-C₄-hydroxyalkyl)₂ ist: R₇₀ H, C₁-C₄-Alkyl, CN, Cl oder SO₃M ist; R₇₉ und R₈₀ unabhängig voneinander H, C₁-C₄-Alkyl, SO₃M, CN, Cl oder O-C₁-C₄-Alkyl darstellen, unter der Voraussetzung, dass mindestens zwei von R₇₈, R₇₉ und R₈₀ SO₃M sind und die dritte Gruppe einen solubilisierenden Charakter aufweist; R₈₁ H, SO₃M, O-C₁-C₄-Alkyl, CN, Cl, COO-C₁-C₄-Alkyl oder CON(C₁-C₄-Alkyl)₂ ist; und r 0 oder 1 ist, und M dessen vorstehende Bedeutung aufweist.

2. Verwendung nach Anspruch 1, worin die Zusammensetzung eine wässrige Textilappretur-Zusammensetzung darstellt und die Menge des in der Zusammensetzung vorliegenden fluoreszierenden Weißmachers von 0,01 bis 3 % reicht; oder die Zusammensetzung eine Reinigungsmittelzusammensetzung darstellt und die Menge des in der Zusammensetzung vorliegenden fluoreszierenden Weißmachers von 0,005 bis 2 % reicht.

3. Verwendung nach Anspruch 1, worin die Zusammensetzung eine wässrige Textilappretur-Zusammensetzung darstellt und der verwendete fluoreszierende Weißmacher eine 4,4'-Bis-(triazinylamino)-stilben-2.2'-disulfonsäure mit der Formel darstellt: worin R₁ und R₂ unabhängig voneinander Phenyl, mono- oder disulfoniertes Phenyl, Phenylamino, mono- oder disulfoniertes Phenylamino, Morpholino, -N(CH₂CH₂OH)₂, -N(CH₃)(CH₂CH₂OH), -NH₂, -N(C₁-C₄-Alkyl)₂, -OCH₃, -Cl, -NH-CH₂CH₂SO₃H oder -NH-CH₂CH₂OH darstellen; und M H, Na, K, Ca, Mg, Ammonium, Mono-, Di-, Tri- oder Tetra-C₁-C₄-alkylammonium, Mono-, Di- oder Tri-C₁-C₄-hydroxyalkylammonium oder Ammonium darstellt, welches mit einer Mischung von C₁-C₄-Alkyl- und C₁-C₄-Hydroxyalkylgruppen di- oder trisubstituiert ist, und
worin die 4,4'-Bis-(triazol-2-yl)stilben-2,2'-disulfonsäure eine solche mit der Formel darstellt: worin R₃ und R₄ unabhängig voneinander H, C₁-C₄-Alkyl, Phenyl oder monosulfoniertes Phenyl sind, und
worin das 4,4'-(Diphenyl)-stilben ein solches mit der Formel ist: und
worin das verwendete 4,4'-Distyryl-biphenyl die Formel aufweist: worin R₅ und R₆ unabhängig voneinander H, SO₃M, SO₂N(C₁-C₄-alkyl)₂, O-(C₁-C₄-Alkyl), CN, Cl, COO(C₁-C₄-Alkyl), CON(C₁-C₄-Alkyl)₂ oder O(CH₂)₃N(+)(CH₃)₂An(-) darstellen, worin An(-) ein Anion einer organischen oder anorganischen Säure ist; und n 0 oder 1 ist, oder worin das 4-Phenyl-4'-benzoxazolylstilben die Formel aufweist: worin R₇ und R₈ unabhängig voneinander H, Cl, C₁-C₄-Alkyl oder SO₂-C₁-C₄-Alkyl sind, und
worin das verwendete Stilbenyl-naphthotriazol ein solches der Formel ist: worin R₉ H oder Cl ist; R₁₀ SO₃M, SO₂N(C₁-C₄-Alkyl)₂, SO₂O-Phenyl oder CN ist:
R₁₁ H oder SO₃M ist, und worin ein verwendetes 4-Styrylstilben ein solches der Formel ist: worin R₁₂ und R₁₃ unabhängig voneinander H, SO₃M, SO₂N(C₁-C₄-Alkyl)₂, O-C₁-C₄-Alkyl), CN, Cl, COO(C₁-C₄-Alkyl), CON(C₁-C₄-Alkyl)₂ oder O(CH₂)₃N(+)-(CH₃)₂An(-) darstellen, und
worin ein verwendetes Bis(benzoxazol-2-yl)-Derivat die Formel aufweist: worin R₁₄ unabhängig voneinander H, C(CH₃)₃, C(CH₃)₂-Phenyl, C₁-C₄-Aryl oder COO-C₁-C₄-Alkyl ist und X -CH=CH- oder eine Gruppe der Formel ist: und worin Bis(Benzimidazol-2-yl)-Derivate der Formel verwendet werden: worin R₁₅ und R₁₆ unabhängig voneinander H, C₁-C₄-Alkyl oder CH₂CH₂OH sind, R₁₇ H oder SO₃M ist; X₁ -CH=CH- oder eine Gruppe der Formel ist: und worin ein Coumarin der Formel verwendet wird: worin R₁₈ H, Cl oder CH₂COOH ist, R₁₉ H, Phenyl, COO-C₁-C₄-Alkyl oder eine Gruppe der Formel ist: und R₂₀ O-C₁-C₄-Alkyl, N(C₁-C₄-Alkyl)₂, NH-CO-C₁-C₄-Alkyl oder eine Gruppe der Formel ist: oder worin R₂₁ H, C₁-C₄-Alkyl oder Phenyl ist, und
worin ein verwendetes Pyrazolin ein solches der Formel ist: worin R₂₂ H, Cl oder N(C₁-C₄-Alkyl)₂ ist; R₂₃ H, Cl, SO₃M, SO₂NH₂, SO₂NH-(C₁-C₄-Alkyl). COO-C₁-C₄-Alkyl, SO₂-C₁-C₄-Alkyl, SO₂NHCH₂CH₂CH₂N(⁺)(CH₃)₃ oder SO₂CH₂CH₂N(+)H(C₁-C₄-Alkyl)₂An (⁻) darstellt, R₂₄ und R₂₅ dieselben oder unterschiedlich sind und jeweils H, C₁-C₄-Alkyl oder Phenyl sind und R₂₆ H oder Cl ist; und
worin ein Naphthalimid der Formel verwendet wird: worin R₂₇ C₁-C₄-Alkyl oder CH₂CH₂CH₂N(⁺)(CH₃)₃ darstellt; R₂₈ O-C₁-C₄-Alkyl, SO₃M oder NH-CO-C₁-C₄-Alkyl ist; und
worin ein Triazinylpyren der Formel verwendet wird: worin R₂₉ jeweils unabhängig voneinander C₁-C₄-Alkoxy darstellt, und
worin ein 2-Styrylbenzoxazol- oder -naphthoxazol-Derivat verwendet wird mit der Formel: worin R₃₁ CN, Cl, COO-C₁-C₄-Alkyl oder Phenyl ist; R₃₂ und R₃₃ die zur Bildung eines anellierten Benzolrings erforderlichen Atome darstellen oder R₃₃ und R₃₅ unabhängig voneinander H oder C₁-C₄-Alkyl sind; und R₃₄ H, C₁-C₄-Alkyl oder Phenyl ist, und
worin ein Benzimidazol-benzofuran-Derivat der Formel verwendet wird: worin R₃₆ C₁-C₄-Alkoxy ist; R₃₇ und R₃₈ unabhängig voneinander C₁-C₄-Alkyl sind;
und worin ein Oxanilid-Derivat der Formel verwendet wird: worin R₃₉ C₁-C₄-Alkoxy ist, R₄₁ C₁-C₄-Alkyl, C₁-C₄-Alkyl-SO₃M oder C₁-C₄-Alkoxy-SO₃M darstellt und R₄₀ und R₄₂ dieselben sind und jeweils Wasserstoff, tert.-Butyl oder SO₃M darstellen.

4. Verwendung nach Anspruch 1, worin die Zusammensetzung eine Textilappretur-Zusammensetzung darstellt und der fluoreszierende Weißmacher verwendet wird:
a) in Mischungen mit Farbstoffen (Farbnuancen) oder Pigmenten;
b) in Mischungen mit Trägern, Benetzungsmitteln, Antioxidationsmitteln, UV-Absorbern und/oder chemischen Bleichmitteln;
c) in Mischung mit Vernetzungs- und Appreturmitteln oder in Kombination mit einem Textilappreturverfahren oder einem Flammschutzfinish. Weichanfühlfinish (soft handle finish), Antiverschmutzungsfinish, Antistatikfinish oder einem antimikrobiellen Finish.

5. Verwendung nach Anspruch 1, worin die Verbindung der Formel (23) die Formel aufweist: oder
worin die Verbindung der Formel (24) die Formel aufweist: worin n die in Anspruch 1 angegebene Bedeutung besitzt;
worin die Verbindung der Formel (26) die Formel aufweist; oder
worin die Verbindung der Formel (27) die Formel aufweist: oder
worin die Verbindung der Formel (30) die Formel aufweist:

6. Verwendung nach Anspruch 1, worin die Verbindung der Formel (56) die Formel (31), (32) oder (34) aufweist, oder worin die Verbindung der Formel (57) die Formel (43), (44), (45) oder (46) aufweist, oder worin die Verbindung der Formel (58) die Formel (40), (41) oder (42) aufweist, jeweils wie in Anspruch 5 definiert.

7. Verwendung nach Anspruch 1, worin die verwendete Zusammensetzung einer Reinigungsmittelzusammensetzung darstellt, umfassend:
i) 5 - 90 % eines anionischen Tensids und/oder eines nichtionischen Tensids;
ii) 5 - 70 % eines Builders;
iii) 0 - 30 % eines Peroxids;
iv) 0 - 10 % eines Peroxidaktivators und/oder 0 - 1 % eines Bleichkatalysators;
v) 0,005 - 2 % mindestens eines fluoreszierenden Weißmachers; welcher Strahlung in dem Wellenlängenbereich 280 - 400 nm absorbiert; und
vi) 0,005 - 10 % eines oder mehrerer Hilfsmittel, jeweils bezogen auf das Gewicht, auf der Basis des Gesamtgewichts des Reinigungsmittels.

8. Stabile, konzentrierte Spülgang-Textilweichmacherzusamensetzung, umfassend 2 bis 25 Gew.-% eines Textilweichmachers und > 0,3 bis 10 Gew.-% eines fluoreszierenden Weißmachers, welcher mit dem Textilweichmacher kompatibel ist, jeweils auf der Basis des Gesamtgewichts der Zusammensetzung, wobei der Rest im wesentlichen Wasser darstellt.

9. Verfahren zur Behandlung eines Textilartikels, umfassend das Auftragen auf einen vorher gewaschenen Artikel einer Textilspülzusammensetzung, umfassend > 0.3 bis 10 Gew.-% eines kationischen, amphoteren oder anionischen fluoreszierenden Weißmachers, auf der Basis des Gesamtgewichts der Zusammensetzung, und wahlweise einen Textilpflegebestandteil, wobei der Rest im wesentlichen Wasser ist.

## Revendications

1. Utilisation d'un agent de blanchiment optique permettant d'améliorer l'indice de protection (IP) d'un matériau en fibres textiles, dans laquelle ledit agent de blanchiment optique absorbe le rayonnement dans la plage de longueurs d'onde allant de 280 à 400 nm, dans une composition qui est
a) une composition aqueuse de finissage textile ;
comprenant au moins un agent de blanchiment optique qui est choisi dans le groupe constitué par l'acide 4,4'-bis-(triazinylamino)-stilbène-2,2'-disulfonique, l'acide 4,4'-bis-(triazol-2-yl)stilbène-2,2'-disulfonique, des 4,4'-(diphényl)-stilbènes, le 4,4'-distyryl-biphényle, le 4-phényl-4'-benzoxazolylstilbène, des stilbénylnaphtotriazoles, le 4-styryl-stilbène, des dérivés bis-(benzoxazol-2-yle), un dérivé bis-(benzimidazol-2-yle), la coumarine, la pyrazoline, le naphtalimide, le triazinyl-pyrène, un dérivé 2-styryl-benzoxazole ou -naphtoxazole, un dérivé benzimidazole-benzofuranne ou oxanilide, ou
b) une composition détergente
comprenant au moins un agent de blanchiment optique, qui est choisi dans le groupe constitué par : dans lesquelles R₄₃ et R₄₄, indépendamment, représentent OH, NH₂, un groupe O-alkyle en C₁-C₄, un groupe O-aryle, un groupe NH-alkyle en C₁-C₄, un groupe N(alkyle en C₁-C₄)₂, un groupe N(alkyle en C₁-C₄) (hydroxyalkyle en C₁-C₄) , un groupe. N(hydroxyalkyle en C₁-C₄) ₂, un groupe NH-aryle, un groupe morpholino, un groupe S-alkyl (aryle) en C₁-C₄, Cl ou OH ; R₄₅ et R₄₆ indépendamment, représentent H, un groupe alkyle en C₁-C₄, un groupe phényle ou un groupe de formule : R₄₇ représente H, Cl ou SO₃M ; R₄₈ représente CN, SO₃M, un groupe S (alkyle en C₁-C₄) ₂ ou un groupe S(aryle)₂ ; R₄₉ représente H, SO₃M, un groupe O-alkyle en C₁-C₄, CN, Cl, un groupe COO-alkyle en C₁-C₄, ou un groupe CON(alkyle en C₁-C₄)₂ ; R₅₀ représente H, un groupe alkyle en C₁-C₄, Cl ou SO₃M ; R₅₁ et R₅₂, indépendamment, représentent H, un groupe alkyle en C₁-C₄, SO₃M, Cl ou un groupe O-alkyle en C₁-C₄ ; R₅₃ représente H ou un groupe alkyle en C₁-C₄; R₅₄ représente H, un groupe alkyle en C₁-C₄, CN, Cl, un groupe COO-alkyle en C₁-C₄, un groupe CON(alkyle en C₁-C₄)₂, un groupe aryle ou un groupe O-aryle ;
et
M représente H, Na, K, Ca, Mg, un ammonium, un mono-, di-, tri- ou tétra-alkylammonium en C₁-C₄, un mono-, di- ou tri-hydroxyalkylammonium en C₁-C₄ ou un ammonium qui est di- ou tri-substitué par un mélange de groupes alkyle en C₁-C₄ et hydroxyalkyle en C₁-C₄, et n vaut 0 ou 1 ;
ou
c) une composition de traitement de tissu après lavage comprenant au moins un agent de blanchiment optique, dans laquelle ledit agent de blanchiment optique est un agent de blanchiment optique bistyrylphényle cationique de formule :
dans laquelle Y représente un groupe arylène, éventuellement substitué par un groupe chloro, méthyle ou méthoxy ; q vaut 1 ou 2 ; R₅₅ représente un atome d'hydrogène, un groupe chloro, un groupe alkyle en C₁-C₄, un groupe alcoxy en C₁-C₄, un groupe cyano ou un groupe alcoxycarbonyle en C₁-C₄ ; R₅₆ et R₅₇ représentent un groupe alkyle en C₁-C₄, un groupe chloroéthyle, un groupe méthoxyéthyle, un groupe bêta-éthoxyéthyle, un groupe bêta-acétoxyéthyle ou bêta-cyanoéthyle, un groupe benzyle ou un groupe phényléthyle ; R₅₈ représente un groupe alkyle en C₁-C₄, un groupe hydroxyalkyle en C₂-C₃, un groupe bêta-hydroxy-gamma-chloropropyle, un groupe bêta-cyanoéthyle ou un groupe alcoxy-carbonyléthyle en C₁-C₄ ; et An (⁻) représente un anion d'un acide organique ou inorganique ; ou,
un agent de blanchiment optique bistyrylphényle cationique de formule : dans laquelle R₅₅ et q ont la même signification que précédemment et Y₁ représente un groupe alkylène en C₂-C₄ ou un groupe hydroxypropylène ; R₅₉ représente un groupe alkyle en C₁-C₄ ou, avec R₆₀ et l'atome d'azote auquel ils sont chacun attachés, R₅₉ forme un cycle pyrrolidine, pipéridine, hexaméthylèneimine ou morpholine ; R₆₀ représente un groupe alkyle en C₁-C₄ ou, conjointement avec R₅₉ et l'atome d'azote auquel ils sont chacun attachés, R₆₀ forme un cycle pyrrolidine, pipéridine, hexaméthylèneimine ou morpholine ; R₆₁ représente un atome d'hydrogène, un groupe alkyle en C₁-C₄, un groupe alcényle en C₃-C₄, un groupe alcoxycarbonylméthyle en C₁-C₄, un groupe benzyle, un groupe hydroxyalkyle en C₂-C₄, un groupe cyanoalkyle en C₂-C₄ ou, conjointement avec R₅₉ et R₆₀ et l'atome d'azote auquel ils sont chacun attachés, R₆₁ forme un cycle pyrrolidine, pipéridine, hexaméthylèneimine ou morpholine ; p vaut 0 ou 1 ; et An(-) représente un anion d'un acide organique ou inorganique ; ou,
un agent de blanchiment optique bistyrylphényle de formule : dans laquelle R₅₅, Y₁, p et q ont la même signification que précédemment et An(-) représente un anion d'un acide organique ou inorganique ; et R₆₂ et R₆₃ indépendamment, représentent un groupe alkyle en C₁-C₄ ou un groupe alcényle en C₂-C₃ ou R₆₂ et R₆₃, conjointement avec l'atome d'azote auquel ils sont attachés, forment un cycle pyrrolidine, pipéridine, hexaméthylèneimine ou morpholine ; R₆₄ représente un atome d'hydrogène, un groupe alkyle en C₁-C₄ ou un groupe alcényle en C₂-C₃ ou R₆₂, R₆₃ et R₆₄, conjointement avec l'atome d'azote auquel ils sont attachés, forment un cycle pyridine ou picoline ; et Z représente un atome de soufre, -SO₂-, -SO₂NH-, un groupe -O-alkylène en C₁-C₄-COO- ou -OCO-, ou, dans laquelle l'agent de blanchiment optique bistyrylphényle cationique a la formule : dans laquelle R₅₅, R₆₂, R₆₃, R₆₄, Y₁, p et q ont la même signification que précédemment et An(-) représente un anion d'un acide organique ou inorganique ; ou,
un agent de blanchiment optique styrène amphotère de formule : dans laquelle R₅₅, R₆₂, R₆₃, Y₁ et q ont la même signification que précédemment et An(-) représente un anion d'un acide organique ou inorganique ; Z₁ représente un atome d'oxygène, un atome de soufre, une liaison directe, -COO-, -CON(R₆₅)- ou -SO₂N (R₆₅) - où R₆₅ représente un atome d'hydrogène, un groupe alkyle en C₁-C₄ ou un groupe cyanoéthyle ; et Q représente -COO- ou -SO₃, et,
dans laquelle l'agent de blanchiment optique oxyde d'amine a la formule : dans laquelle q a la même signification que précédemment et B représente un radical d'azurant optique choisi parmi un 4,4'-distyrylbiphényle, un 4,4'-divinyl-stilbène, et un 1,4'-distyrylbenzène, chacun étant éventuellement substitué par un à quatre substituants choisis parmi un atome d'halogène, un groupe alkyle en C₁-C₄, un groupe hydroxyalkyle en C₁-C₄, un groupe halogénoalkyle en C₁-C₄, un groupe cyanoalkyle en C₁-C₄, un groupe alcoxy en C₁-C₄-alkyle en C₁-C₄, un groupe phényl-alkyle en C₁-C₄, un groupe carboxy-alkyle en C₁-C₄, un groupe carb-alcoxy en -C₁-C₄-alkyle en C₁-C₄, un groupe alcényle en C₁-C₄, un groupe cycloalkyle en C₅-C₈, un groupe alcoxy en C₁-C₄, un groupe alcénoxy en C₁-C₄, un groupe alcoxycarbonyle en C₁-C₄, un groupe carbamoyle, un groupe cyano, un groupe alkylsulfonyle en C₁-C₄, un groupe phénylsulfonyle, un groupe alcoxysulfonyle en C₁-C₄, un groupe sulfamoyle, un groupe hydroxyle, un groupe carboxyle, un groupe sulfo et un groupe trifluorométhyle ; Z₂ représente une liaison directe entre B et Y₂, un atome d'oxygène, un atome de soufre, -SO₂-, -SO₂-O-, -COO-, -CON(R₆₈) ou -SO₂N(R₆₈)- où R₆₈ représente un atome d'hydrogène ou un groupe alkyle en C₁-C₄ éventuellement substitué par un atome d'halogène, un groupe cyano, un groupe hydroxyle, un groupe carbalcoxy en C₂-C₅, un groupe alcoxy en C₁-C₄, un groupe phényle, un groupe chlorophényle, un groupe méthylphényle, un groupe méthoxyphényle, un groupe carbamoyle ou un groupe sulfamoyle ; Y₂ représente un groupe alkylène en C₂-C₄ ou un groupe alkylénoxy en C₂-C₄-alkylène en C₂-C₄, chacun étant éventuellement substitué par un atome d'halogène, un groupe hydroxyle, un groupe carbalcoxy en C₂-C₅, un groupe alcoxy en C₁-C₄, un groupe phényle, un groupe chlorophényle, un groupe méthylphényle, un groupe méthoxyphényle, un groupe carbamoyle ou un groupe sulfamoyle ; et R₆₆ et R₆₇, indépendamment, représentent un groupe cycloalkyle en C₅-C₈, un groupe alkyle en C₁-C₄ ou un groupe phényle, chacun étant éventuellement substitué par un atome d'halogène, un groupe hydroxyle, un groupe carbalcoxy en C₂-C₅, un groupe alcoxy en C₁-C₄, un groupe phényle, un groupe chlorophényle, un groupe méthylphényle, un groupe méthoxyphényle, un groupe carbamoyle ou un groupe sulfamoyle ; où, dans tous les groupes carbamoyle ou sulfamoyle, l'atome d'azote est éventuellement substitué par un ou deux groupes alkyle en C₁-C₄, hydroxyalkyle en C₁-C₄, cyanoalkyle en C₂-C₅, halogénoalkyle en C₁-C₄, benzyle ou phényle, ou,
un agent de blanchiment optique cationique de formule : dans laquelle Y₂ et q ont la même signification que précédemment, et B₁ représente un radical d'azurant optique ; Z₃ représente une liaison directe, un groupe -SO₂-alkylénoxy en C₂-C₄, un groupe -O₂-alkylène en C₂-C₄-COO-, -SO₂-, -COO-, un groupe -SO₂-alkylène en C₂-C₄-CON (R₇₅)- ou -SO₂N (R₇₅)- où R₇₅ représente un atome d'hydrogène ou un groupe alkyle en C₁-C₄ éventuellement substitué par un groupe hydroxyle, un atome d'halogène ou un groupe cyano ; R₇₀ représente un groupe alkyle en C₁-C₄ ou un groupe alcényle en C₁-C₄, chacun étant éventuellement substitué par un atome d'halogène, un groupe cyano, un groupe hydroxy, un groupe alcoxycarbonyle en C₁-C₄ ou un groupe alkylcarbonyloxy en C₁-C₄, ou R₇₀ représente un groupe benzyle éventuellement substitué par un atome d'halogène, un groupe alkyle en C₁-C₄ ou un groupe alcoxy en C₁-C₄, ou R₇₀, conjointement avec R₇₁ ou Z₃, forme un radical pyrrolidine, pipéridine ou morpholine ; R₇₁ représente un groupe alkyle en C₁-C₄ ou un groupe alcényle en C₂-C₄, chacun étant éventuellement substitué par un atome d'halogène, un groupe cyano, un groupe hydroxy, un groupe alcoxycarbonyle en C₁-C₄ ou un groupe alkylcarbonyloxy en C₁-C₄, ou R₇₁ représente un groupe benzyle, éventuellement substitué par un atome d'halogène, un groupe alkyle en C₁-C₄ ou un groupe alcoxy en C₁-C₄, ou R₇₁, conjointement avec R₇₀, forme un radical pyrrolidine, pipéridine ou morpholine ; R₇₂ représente un groupe alkyle en C₁-C₄, R₇₃ représente un atome d'hydrogène ou
un groupe alkyle en C₁-C₄, éventuellement substitué par un groupe cyano, un groupe hydroxy, un groupe alcoxycarbonyle en C₁-C₄ ou un groupe alkylcarbonyloxy en C₁-C₄ ; et R₇₄ représente un groupe alkyle en C₁-C₄,
ou,
dans laquelle ledit agent de blanchiment optique est un agent de blanchiment optique anionique bis(triazinyl)diaminostilbène de formule : ou un agent de blanchiment optique anionique dibenzofuranylbiphényle de formule : ou un agent optique bistyrylphényle anionique de formule : dans laquelle R₇₆ représente un groupe phényle éventuellement substitué par un ou deux groupes SO₃M et R₇₇ représente un groupe NH-alkyle en C₁-C₄, un groupe N (alkyle en C₁-C₄)₂, un groupe NH-alcoxy en C₁-C₄, un groupe N (alcoxy en C₁-C₄) ₂, un groupe N (alkyle en C₁-C₄)(hydroxyalkyle en C₁-C₄), un groupe N (hydroxyalkyle en C₁-C₄) ₂ ; R₇₀ représente H, un groupe alkyle en C₁-C₄, CN, Cl ou SO₃M ; R₇₉ et R₈₀, indépendamment, représentent H, un groupe alkyle en C₁-C₄, SO₃M, CN, Cl ou un groupe O-alkyle en C₁-C₄, à condition qu'au moins deux de R₇₈, R₇₉ et R₈₀ représentent SO₃M et que le troisième groupe ait un caractère solubilisant ; R₈₁ représente H, SO₃M, un groupe O-alkyle en C₁-C₄, CN, Cl, un groupe COO-alkyle en C₁-C₄, ou un groupe CON(alkyle en C₁-C₄) ₂ ; et r vaut 0 ou 1, et M a la même signification que précédemment.

2. Utilisation selon la revendication 1, dans laquelle la composition est une composition aqueuse de finissage textile et la quantité d'agent de blanchiment optique présente dans la composition se situe dans la plage allant de 0,01 à 3 % ; ou la composition est une composition détergente et la quantité d'agent de blanchiment optique présente dans la composition se situe dans la plage allant de 0,005 à 2 %.

3. Utilisation selon la revendication 1, dans laquelle la composition est une composition aqueuse de finissage textile et l'agent de blanchiment optique utilisé est l'acide 4,4'-bis-(triazinylamino)-stilbène-2,2'-disulfonique, ayant la formule : dans laquelle R₁ et R₂, indépendamment, représentent un groupe phényle, un groupe phényle mono- ou disulfoné, un groupe phénylamino, un groupe phénylamino mono- ou disulfoné, un groupe morpholino, -N (CH₂CH₂OH)₂, -N(CH₃) (CH₂CH₂OH), -NH₂, un groupe -N(alkyle en C₁-C₄)₂, -OCH₃, -Cl, -NH-CH₂CH₂SO₃H ou -NH-CH₂CH₂OH ; et M représente H, Na, K, Ca, Mg, un ammonium, un mono-, di-, tri- ou tétra-alkylammonium en C₁-C₄, un mono-, di- ou tri-hydroxyalkylammonium en C₁-C₄ ou un ammonium qui est di- ou tri-substitué par un mélange de groupes alkyle en C₁-C₄ et hydroxyalkyle en C₁-C₄, et
dans laquelle l'acide 4,4'-bis-(triazol-2-yl)-stilbène-2,2'-disulfonique est celui ayant la formule : dans laquelle R₃ et R₄, indépendamment, représentent H, un groupe alkyle en C₁-C₄, un groupe phényle ou un groupe phényle monosulfoné et, dans laquelle le 4,4'-(diphényl)-stilbène est celui ayant la formule : et,
dans laquelle le 4,4'-distyryl-biphényle utilisé a la formule : dans laquelle R₅ et R₆, indépendamment, représentent H, SO₃M, un groupe SO₂N (alkyle en C₁-C₄)₂, un groupe O-(alkyle en C₁-C₄), CN, Cl, un groupe COO(alkyle en C₁-C₄), un groupe CON(alkyle en C₁-C₄)₂ ou O (CH₂) ₃N (+) (CH₃) ₂An (-) , où An (-) représente un anion d' un acide organique ou inorganique ; et n vaut 0 ou 1, ou dans laquelle le 4-phényl-4'-benzoxazolyl-stilbène a la formule : dans laquelle R₇ et R₈, indépendamment, représentent H, Cl, un groupe alkyle en C₁-C₄ ou un groupe SO₂-alkyle en C₁-C₄, et dans laquelle un stilbényl-naphtotriazole utilisé est celui de formule : dans laquelle R₉ représente H ou Cl; R₁₀ représente SO₃M, un groupe SO₂N (alkyle en C₁-C₄)₂, ou un groupe SO₂O-phényle ou CN ; R₁₁ représente H ou SO₃M, et dans laquelle un 4-styryl-stilbène utilisé est celui de formule : dans laquelle R₁₂ et R₁₃, indépendamment, représentent H, SO₃M, un groupe SO₂N (alkyle en C₁-C₄)₂, un groupe O-(alkyle en C₁-C₄), CN, Cl, un groupe COO(alkyle en C₁-C₄), un groupe CON(alkyle en C₁-C₄) ₂ ou O(CH₂)₃N(+)(CH₃)₂An(-), et dans laquelle un dérivé bis-(benzoxazol-2-yle) utilisé a la formule : dans laquelle R₁₄, indépendamment, représente H, C(CH₃)₃, un groupe C(CH₃)₂-phényle, un groupe alkyle en C₁-C₄ ou un groupe COO-alkyle en C₁-C₄, et X représente -CH=CH- ou un groupe de formule : et
dans laquelle un dérivé bis-(benzimidazol-2-yle) est utilisé de formule : dans laquelle R₁₅ et R₁₆, indépendamment, représentent H, un groupe alkyle en C₁-C₄ ou CH₂CH₂OH ; R₁₇ représente H ou SO₃M ; X₁ représente -CH=CH- ou un groupe de formule : et dans laquelle une coumarine est utilisée de formule : dans laquelle R₁₈ représente H, Cl ou CH₂COOH, R₁₉ représente H, un groupe phényle, un groupe COO-alkyle en C₁-C₄ ou un groupe de formule : et R₂₀ représente un groupe O-alkyle en C₁-C₄, un groupe N(alkyle en C₁-C₄)₂, un groupe NH-CO-alkyle en C₁-C₄ ou un groupe de formule : ou
dans laquelle R₂₁ représente H, un groupe alkyle en C₁-C₄ ou un groupe phényle, et
dans laquelle une pyrazoline utilisée est celle ayant la formule : dans laquelle R₂₂ représente H, Cl, ou un groupe N(alkyle en C₁-C₄) ₂, R₂₃ représente H, Cl, SO₃M, SO₂NH₂, un groupe SO₂NH-(alkyle en C₁-C₄), un groupe COO-alkyle en C₁-C₄, un groupe SO₂-alkyle en C₁-C₄, SO₂NHCH₂CH₂CH₂N (⁺) (CH₃) ₃ ou un groupe SO₂CH₂CH₂N(⁺) H (alkyle en C₁-C₄)₂An (⁻), R₂₄ et R₂₅ sont identiques ou différents et chacun représente H, Cl, un groupe alkyle en C₁-C₄ ou un groupe phényle et R₂₆ représente H ou Cl ; et
dans laquelle un naphtalimide est utilisé de formule : dans laquelle R₂₇ représente un groupe alkyle en C₁-C₄ ou CH₂CH₂CH₂N(⁺) (CH₃)₃ ; R₂₈ représente un groupe O-alkyle en C₁-C₄, SO₃M ou un groupe NH-CO-alkyle en C₁-C₄ ; et
dans laquelle un triazinyl-pyrène est utilisé de formule: dans laquelle chaque R₂₉, indépendamment, représente un groupe alcoxy en C₁-C₄, et
dans laquelle un dérivé 2-styryl-benzoxazole ou -naphtoxazole est utilisé ayant la formule : dans laquelle R₃₁ représente CN, Cl, un groupe COO-alkyle en C₁-C₄ ou un groupe phényle ; R₃₂ et R₃₃ représentent les atomes requis pour former un cycle benzène condensé ou R₃₃ et R₃₅, indépendamment, représentent H ou un groupe alkyle en C₁-C₄ ; et R₃₄ représente H, un groupe alkyle en C₁-C₄ ou un groupe phényle, et,
dans laquelle un dérivé benzimidazole-benzofuranne est utilisé ayant la formule : dans laquelle R₃₆ représente un groupe alcoxy en C₁-C₄ ; R₃₇ et R₃₈, indépendamment, représentent un groupe alkyle en C₁-C₄;
et dans laquelle un dérivé oxanilide est utilisé ayant la formule : dans laquelle R₃₉ représente un groupe alcoxy en C₁-C₄, R₄₁ représente un groupe alkyle en C₁-C₄, un groupe alkyle en C₁-C₄-SO₃M ou un groupe alcoxy en C₁-C₄-SO₃M et R₄₀ et R₄₂ sont identiques et chacun représente un atome d'hydrogène, un groupe tert-butyle ou SO₃M.

4. Utilisation selon la revendication 1, dans laquelle la composition est une composition de finissage textile et l'agent de blanchiment optique est utilisé :
a) dans des mélanges avec des colorants (coloration légère) ou des pigments ;
b) dans des mélange avec des véhicules, des agents mouillants, des antioxydants, des absorbants d'UV et/ou des agents de blanchiment chimique ; ou
c) en mélange avec des agents de réticulation ou de finissage ou en combinaison avec un procédé de finissage textile ou un apprêt ignifugeant, un apprêt pour la douceur, un apprêt antisalissures, un apprêt antistatique ou un apprêt antimicrobien.

5. Utilisation selon la revendication 1, dans laquelle le composé de formule (23) a la formule : ou
dans laquelle le composé de formule (24) à la formule : dans laquelle n est tel que défini dans la revendication 1 ;
dans laquelle le composé de formule (26) a la formule : ou
dans laquelle le composé de formule (27) a la formule : ou
dans laquelle le composé de formule (30) a la formule :

6. Utilisation selon la revendication 1, dans laquelle le composé de formule (56) a la formule (31), (32) ou (34), ou dans laquelle le composé de formule (57) a la formule (43), (44), (45) ou (46) ou dans laquelle le composé de formule (58) a la formule (40), (41), ou (42), chacune étant telle que définie dans la revendication 5.

7. Utilisation selon la revendication 1, dans laquelle la composition utilisée est une composition détergente comprenant :
i) de 5 à 90 % d'un tensioactif anionique et/ou d'un tensioactif non ionique ;
ii) de 5 à 70 % d'un adjuvant ;
iii) de 0 à 30 % d'un peroxyde ;
iv) de 0 à 10 % d'un. activateur de peroxyde et/ou de 0 à 1 % d'un catalyseur de blanchiment ;
v) de 0,005 à 2 % d'au moins un agent de blanchiment optique qui absorbe le rayonnement dans la plage de longueurs d'onde allant de 280 à 400 nm ; et
vi) de 0,005 à 10 % d'un ou plusieurs auxiliaires, chacun en poids, par rapport au poids total du détergent.

8. Composition adoucissante de tissu pour cycle de rinçage concentrée et stable comprenant de 2 à 25 % en poids d'un agent adoucissant de tissu, et > 0,3 à 10 % en poids d'un agent de blanchiment optique qui est compatible avec l'agent adoucissant de tissu, chacun par rapport au poids total de la composition, le reste étant essentiellement de l'eau.

9. Procédé pour le traitement d'un article textile, comprenant une étape d'application, sur un article préalablement lavé, d'une composition de rinçage de tissu comprenant > 0,3 à 10 % en poids d'un agent de blanchiment optique cationique, amphotère ou anionique, par rapport au poids total de la composition, et éventuellement d'un ingrédient de traitement de tissu, le reste étant essentiellement de l'eau.
